# EUROPEAN PATENT SPECIFICATION

(11) **EP 4 441 178 B1**
(45) Date of publication and mention of the grant of the patent: **14.05.2025**
(21) Application number: 22829708.1
(22) Date of filing: 01.12.2022
(51) Int. Cl.: C10M 155/04, C08L 43/00, C10M 157/10, C08F 238/00, C08F 301/00

(54) **LUBRICANT COMPOSITIONS**
SCHMIERMITTELZUSAMMENSETZUNGEN
COMPOSITIONS LUBRIFIANTES

(30) Priority: 03.12.2021 EP 21306699
(43) Date of publication of application: 09.10.2024
(73) Proprietor: TotalEnergies OneTech, 92400 Courbevoie (FR)
(72) Inventor: BRIAND, Fanny, 69360 SOLAIZE (FR)
(74) Representative: Bandpay & Greuter
(86) International application number: PCT/EP2022/083980
(87) International publication number: WO 2023/099634

(56) References cited:
- US-A1- 2018 023 028
- US-A1- 2019 382 679
- US-A1- 2021 309 930

## Description

The present invention is directed to lubricant compositions and additive compositions comprising boronic ester-modified polyalkyl(meth)acrylate copolymers. A simple, cost-effective method for their preparation is also disclosed.

Global government vehicle regulations demand ever better fuel economy to reduce greenhouse gas emissions and conserve fossil fuels. There is an increasing demand for more fuel-efficient vehicles in order to meet the targets regarding CO₂ emissions. Therefore, any incremental improvement in fuel economy (FE) is of great importance in the automotive sector.

Lubricants are playing an important role in reducing a vehicle's fuel consumption and there is a continuing need for improvements in fuel economy performance.

Lubricant properties are typically improved by the addition of additives to lubricating oils. Viscosity index (VI) improvers are generally added to a lubricant to improve its thickening efficiency and to protect the engine as they are applied between the surfaces of moving parts, notably metal surfaces.

The thickening efficiency of a VI improver is specified by its KV100 (kinematic viscosity at 100°C) at a given treat rate. The thickening effect of a polymer increases as its hydrodynamic volume in the oil increases. Increasing temperature increases the solvency of the oil, which, in turn, promotes the uncoiling of the polymer and results in a larger hydrodynamic volume.

The hydrodynamic volume of a polymer in solution depends on many parameters, such as for example the polymer chain length and composition. The longer a polymer chain, the higher is usually the weight-average molecular weight M_{w}.

The drawback of using VI improvers with a high molecular weight is that they undergo significant and irreversible degradation under mechanical stress. Such degraded polymers then experience a decline in its thickening properties that goes along with an irreversible drop in the viscosity of the lubricant.

One way to overcome this disadvantage is to prepare polymers of lower molecular weight that can associate under higher temperatures by exchanging chemical bonds in a thermo-reversible way.

### State of the Art

Patent applications US 2017/008989, US 2017/009176 and US 2018/0023028 disclose a composition resulting from the mixing of at least one copolymer A1 resulting from the copolymerization of at least one monomer functionalized by diol functional groups and of at least one compound A2 comprising at least two boronic ester functional groups. These compounds can associate and exchange chemical bonds in a thermo-reversible way. The polymers according to the present invention are not described.

WO 2019/171006 is directed to a composition resulting from the mixing of at least one comb polymer polydiol A1 and at least one compound A2 comprising at least two boronic ester functions. The polymers according to the present invention are not described.

WO 2019/171007 is directed to a composition resulting from the mixing of at least one polydiol compound A1 and at least one comb polymer A2 comprising at least two boronic ester functions. The polymers according to the present invention are not described.

WO 2019/224491, WO 2019/224492, WO 2019/224493 and WO 2019/224494 are directed to a composition resulting from the mixing of at least one oligomer A1, functionalized with diols and optionally comprising repeat units from at least one styrene monomer, and at least one compound A2 comprising at least two boronic ester functions. The polymers according to the present invention are not described.

It was now an object of the present invention to provide thermo-associative polymers that can be used as viscosity index improvers in lubricating oil compositions and that are stable over a broad temperature range. Such polymers should be usable at low treat rates.

Additionally, the synthesis of such polymers should be simple and easy to upscale, and the starting materials should be commercially available.

The Applicant set itself the objective of preparing lubricant compositions based on novel thermoassociative copolymer mixtures which have improved properties when compared with the copolymer mixtures of the prior art. The Applicant also set itself the objective of preparing lubricant compositions based on novel thermoassociative copolymer mixtures which are easy to prepare and are not too costly.

This objective is achieved by means of novel rheological additives which can associate, optionally to form a gel, and which can be exchanged. The additives of the present invention have the advantage of thickening the medium in which they are dispersed, and they maintain this advantage at high temperatures, for instance up to 150°C. These additives show resistance to chemical degradation during a temperature increase when compared with the additives of the prior art. Lubricant compositions comprising them show better stability of their cycling performance and better reproducibility of the lubricant properties over time.

This characteristic results from the combined use of two particular compounds, a copolymer bearing diol functions and a copolymer comprising boronic ester functions.

It is possible, by means of the compositions of the invention, to provide lubricant compositions which have good lubricant properties during the start-up phases of an engine (cold phase) and good lubricant properties when the engine is running at its service temperature (hot phase). These lubricant compositions make it possible to reduce the fuel consumption of a vehicle in which they are used. They allow better resistance to mechanical degradation than the compositions of the prior art.

### Summary of the invention

The invention is based on the introduction into a base oil, of a thermoassociative copolymer mixture comprising at least a boronic ester-modified polyalkyl (meth)acrylate copolymer **A** and a diol functionalized polyalkyl (meth)acrylate copolymer **B.**

The invention relates to a lubricating oil composition, comprising at least:
- more than 60% by weight, based on the total weight of the lubricating composition, of a base oil,
- a boronic ester-modified polyalkyl (meth)acrylate copolymer **A,** comprising 2 mol% to 6 mol% of maleic acid anhydride, and 2 mol% to 6 mol% of an aminophenylboronic acid ester of general formula (I) Wherein the definition of R1, R2 and n is detailed below
   and
- a diol functionalized polyalkyl (meth)acrylate copolymer **B** comprising from 90% to 98% molar of C1-30 alkyl (meth)acrylates, and from 2% to 10% molar of a C2-30 α,β-di-hydroxyalkyl (meth)acrylate.

A second object of the invention relates to a lubricating oil composition, comprising at least:
- more than 60% by weight, based on the total weight of the lubricating oil composition, of a base oil,
- a boronic ester-modified polyalkyl (meth)acrylate copolymer **A** comprising from 1% to 3% by weight of copolymerized or grafted maleic acid anhydride, and from 2% to 6% by weight of an aminophenylboronic acid ester of general formula (I) Wherein the definition of R1, R2 and n is detailed below
   and
- a diol functionalized polyalkyl (meth)acrylate copolymer **B** comprising from 1% to 6% by weight of a diol selected from C2-30 α,β-dihydroxyalkyl (meth)acrylates.

According to a favorite embodiment, the lubricating oil composition, comprises at least:
- more than 60% by weight, based on the total weight of the lubricating composition, of a base oil,
- a boronic ester-modified polyalkyl (meth)acrylate copolymer **A,** comprising:

| | |
|---|---|
| (a1) | 15% to 40% by weight of C1-4 alkyl (meth)acrylates, preferably selected from methyl methacrylate and butyl methacrylate, more preferably butyl methacrylate; |
| (a2) | 45% to 80% by weight of C10-30 alkyl (meth)acrylates, preferably a mixture of C12-15 alkyl (meth)acrylates and C16-20 alkyl (meth)acrylates, more preferably a mixture of C12-14 alkyl (meth)acrylates and C16-18 alkyl (meth)acrylates; |
| (a3) | 0% to 20% by weight of comonomers; |
| (a4) | 1% to 3% by weight of copolymerized or grafted maleic acid anhydride; and |
| (a5) | 2% to 6% by weight of an aminophenylboronic acid ester of general formula (I) |

Wherein the definition of R1, R2 and n is detailed below
and
- a diol functionalized polyalkyl (meth)acrylate copolymer **B** comprising
(b1) 15% to 40% by weight of C1-4 alkyl (meth)acrylates, preferably selected from methyl methacrylate and butyl methacrylate, more preferably butyl methacrylate;
(b2) 45% to 80% by weight of C10-30 alkyl (meth)acrylates, preferably a mixture of C12-15 alkyl (meth)acrylates and C16-20 alkyl (meth)acrylates, more preferably a mixture of C12-14 alkyl (meth)acrylates and C16-18 alkyl (meth)acrylates;
(b3) 0% to 20% by weight of comonomers; and
(b4) 1% to 6% by weight of a diol selected from C2-30 α,β-di-hydroxyalkyl (meth)acrylate preferably C2-10 α,β-dihydroxyalkyl (meth)acrylates, preferably selected from the group consisting of 2,3-dihydroxypropyl methacrylate and 5,6-dihydroxyhexyl methacrylate.

According to a favorite embodiment, in the aminophenylboronic acid ester of general formula (I):
**n** denotes an integer from 0 to 12,
**R¹** and **R²** are independently selected from the group consisting of hydrogen and C1-12 alkyl, or
**R¹** together with **R²** form a ring of general formula (IIa)
wherein **R³, R⁴, R⁵** and **R⁶** are independently selected from the group consisting of H and C1-12 alkyl and the stars "*" represent the bonds to the oxygen atoms, or
**R¹** together with **R²** form a ring of general formula (IIb)
wherein **R³** and **R⁶** are independently selected from the group consisting of H and C1-12 alkyl and the stars "*" represent the bonds to the oxygen atoms, or
**R¹** together with **R²** form a ring of general formula (IIc)
wherein R⁷ denotes a hydrogen atom or C1-4 alkyl and the stars "*" represent the bonds to the oxygen atoms.

According to a favorite embodiment, the lubricating oil composition comprises at least:
- from more than 60% to 99.8 % by weight of a base oil;
- from 0.1% to 10% by weight of the boronic ester-modified polyalkyl (meth)acrylate copolymer **A,** and
- from 0.1% to 10% by weight of the diol functionalized polyalkyl (meth)acrylate copolymer **B**

Another object of the invention is an additive composition which can be used for the preparation of the lubricating oil composition, comprising at least:
(A) 0.1% to 25% by weight of a boronic ester-modified polyalkyl (meth)acrylate copolymer **A,**
(B) 0.1% to 25% by weight of a diol functionalized polyalkyl (meth)acrylate copolymer **B,**
(C) 40% to 60% by weight of a base oil; and
(D) 0.1% to 30% by weight of at least one additive selected from the group consisting of conventional VI improvers, dispersants, defoamers, detergents, antioxidants, pour point depressants, antiwear additives, extreme pressure additives, friction modifiers, anticorrosion additives, dyes and mixtures thereof.

Another object of the invention is a method of thickening a lubricating oil composition, comprising the steps of:
(i) preparing a boronic ester-modified polyalkyl (meth)acrylate copolymer **A;**
(ii) mixing the boronic ester-modified polyalkyl (meth)acrylate copolymer **A** of step (i) with a diol functionalized polyalkyl (meth)acrylate copolymer **B** to form a thermo-associative polymer mixture; and
(iii) introducing the polymer mixture of step (ii) into a lubricating oil composition, Wherein the boronic ester-modified polyalkyl (meth)acrylate copolymer **A,** the diol functionalized polyalkyl (meth)acrylate copolymer **B** and the lubricating oil composition are as defined above and in details here-under.

The invention is also directed to the use of the lubricating oil composition or the additive oil composition for reducing the fuel consumption of vehicles.

The invention is further directed to a process for reducing the energy losses by mechanical part friction, comprising at least one step of placing a mechanical part in contact with the lubricating oil composition.

The invention is also directed to a process for reducing the fuel consumption of a vehicle, comprising at least one step of placing a mechanical part of the vehicle engine in contact with the lubricating oil composition.

### Detailed Description of the invention

The expression "consists essentially of" followed by one or more features means that, besides the components or steps explicitly listed, components or steps which do not significantly modify the properties and features of the invention may be included in the process or the material of the invention.

The expression "between X and Y" includes the limits, unless explicitly mentioned otherwise. This expression thus means that the targeted range comprises the values X and Y and all the values ranging from X to Y.

The term "copolymer" means a linear or branched oligomer or macromolecule having a sequence formed from several repeating units (or monomer units), of which at least two units have a different chemical structure.

The term "monomer unit" or "monomer" means a molecule that is capable of being converted into an oligomer or a macromolecule by combination with itself or with other molecules of the same type. A monomer denotes the smallest constituent unit whose repetition leads to an oligomer or a macromolecule.

In the context of this invention, the expression: "a copolymer comprising monomer X" (for example a copolymer comprising maleic acid anhydride) means a copolymer comprising repeating units resulting from the copolymerization of monomers X with other monomers. The same applies to each and every monomer and copolymer cited in this application.

In the context of the invention the expression "a polymer" or "the polymer" can be used to designate a copolymer resulting from the copolymerization of two or more different monomers.

### The boronic ester-modified polyalkyl (meth)acrylate copolymer A

The first copolymer of the thermoassociative copolymer mixture is a boronic ester-modified polyalkyl (meth)acrylate copolymer **A,** comprising maleic acid anhydride, and an aminophenylboronic acid ester of general formula (I) wherein
**n** denotes an integer from 0 to 12, **R¹** and **R²** are independently selected from the group consisting of hydrogen and C1-12 alkyl, or **R¹** together with **R²** form a ring of general formula (IIa)
wherein **R³, R⁴, R⁵** and **R⁶** are independently selected from the group consisting of H and C1-12 alkyl and the stars "*" represent the bonds to the oxygen atoms, or
**R¹** together with **R²** form a ring of general formula (IIb)
wherein **R³** and **R⁶** are independently selected from the group consisting of H and C1-12 alkyl and the stars "*" represent the bonds to the oxygen atoms, or
**R¹** together with **R²** form a ring of general formula (IIc)
wherein **R⁷** denotes a hydrogen atom or C1-4 alkyl and the stars "*" represent the bonds to the oxygen atoms.

According to a favorite embodiment of the present invention, the boronic ester-modified polyalkyl (meth)acrylate copolymer **A** comprises maleic acid anhydride, at least an aminophenylboronic acid ester of general formula (I), and C1-30 alkyl (meth)acrylates.

According to a more favorite embodiment of the present invention, the maleic acid anhydride, the aminophenylboronic acid ester(s) of general formula (I), and the C1-30 alkyl (meth)acrylates represent from 95% to 100% by weight of the monomers composing copolymer **A,** preferably from 98% to 100% by weight, even more preferably they represent 100% by weight of the monomers composing copolymer **A.**

According to a first embodiment of the invention, the first copolymer of the thermoassociative copolymer mixture is a boronic ester-modified polyalkyl (meth)acrylate copolymer **A,** comprising 2 mol% to 6 mol% of maleic acid anhydride, and 2 mol% to 6 mol% of an aminophenylboronic acid ester of general formula (I)

Wherein **R¹, R²** and n are as defined above and in detail above and here-under. According to a favorite variant of this embodiment of the present invention, the boronic ester-modified polyalkyl (meth)acrylate copolymer **A** comprises from 2 mol% to 6 mol% of maleic acid anhydride, from 2 mol% to 6 mol% of an aminophenylboronic acid ester of general formula (I), and from 75% to 96% molar of C1-30 alkyl (meth)acrylates.

According to another favorite embodiment of the present invention, the boronic ester-modified polyalkyl (meth)acrylate copolymer **A,** comprises:

| | |
|---|---|
| (a1) | 15% to 40% by weight of C1-4 alkyl (meth)acrylates, preferably selected from methyl methacrylate and butyl methacrylate, more preferably butyl methacrylate; |
| (a2) | 45% to 80% by weight of C10-30 alkyl (meth)acrylates, preferably a mixture of C12-15 alkyl (meth)acrylates and C16-20 alkyl (meth)acrylates, more preferably a mixture of C12-14 alkyl (meth)acrylates and C16-18 alkyl (meth)acrylates; |
| (a3) | 0% to 20% by weight of comonomers; |
| (a4) | 1% to 3% by weight of copolymerized or grafted maleic acid anhydride; and |
| (a5) | 2% to 6% by weight of an aminophenylboronic acid ester of general formula (I) |

wherein n denotes an integer from 0 to 12, **R¹** and **R**² are independently selected from the group consisting of hydrogen and C1-12 alkyl, or **R¹** together with **R²** form a ring of general formula (IIa)
wherein **R³, R⁴, R⁵** and **R⁶** are independently selected from the group consisting of H and C1-12 alkyl and the stars "*" represent the bonds to the oxygen atoms, or
**R¹** together with **R²** form a ring of general formula (IIb)
wherein **R³** and **R⁶** are independently selected from the group consisting of H and C1-12 alkyl and the stars "*" represent the bonds to the oxygen atoms, or
**R¹** together with **R²** form a ring of general formula (IIc)
wherein **R⁷** denotes a hydrogen atom or C1-4 alkyl and the stars "*" represent the bonds to the oxygen atoms.

The content of each component (a1), (a2), (a3), (a4) and (a5) is based on the total composition of the boronic ester-modified polyalkyl (meth)acrylates **A.** In a particular embodiment, the proportions of components (a1), (a2), (a3), (a4) and (a5) add up to 100% by weight.

According to a favorite embodiment of the present invention, in the boronic ester-modified polyalkyl (meth)acrylates **A,** the C10-30 alkyl (meth)acrylates are a mixture of C12-15 alkyl (meth)acrylates and C16-20 alkyl (meth)acrylates in a weight ratio of 2:1 to 3:1.

According to a favorite embodiment of the present invention, in the boronic ester-modified polyalkyl (meth)acrylate **A** as defined further above, in general formula (I), n denotes an integer 1 or 2 and **R¹** together with **R²** form a ring of general formula (IIa) wherein **R³** and **R⁶** are independently selected from the group consisting of H and C1-3 alkyl, **R⁴** and **R⁵** are independently selected from the group consisting of H and C1-12 alkyl, and the stars "*" represent the bonds to the oxygen atoms.

In the boronic ester-modified polyalkyl (meth)acrylate copolymer **A** as defined further above, in general formula (I), the amino function can be in the ortho, meta or para position with regards to the bore substituent. According to a favorite embodiment of the present invention the amino function is in the ortho or para position with regards to the bore substituent, even more preferably in the para position.

The weight-average molecular weight of the boronic ester-modified polyalkyl (meth)acrylates **A** used in the lubricating composition according to the present invention is preferably in the range of 50,000 to 800,000 g/mol, more preferably in the range of 100,000 to 600,000 g/mol. The number-average molecular weight of the polyalkyl(meth)acrylate polymers according to the present invention is preferably in the range of 30,000 to 100,000 g/mol, more preferably in the range of 40,000 to 80,000 g/mol.

Preferably, the polyalkyl(meth)acrylate copolymers **A** used in the lubricating composition according to the present invention have a polydipersity index (PDI) M_{w}/Mₙ in the range of 1 to 10, more preferably in the range of 2 to 6.

M_{w} and Mₙ are determined by size exclusion chromatography (SEC) using commercially available polymethylmethacrylate standards. The determination was done by gel permeation chromatography with THF as eluent.

The term "(meth)acrylates" refers to both, esters of acrylic acid and esters of methacrylic acid. Esters of methacrylic acid are preferred.

The C1-4 alkyl (meth)acrylates for use in accordance with the invention are esters of (meth)acrylic acid and straight chain or branched alcohols having 1 to 4 carbon atoms. The term "C1-4 alkyl (meth)acrylates" encompasses individual (meth)acrylic esters with an alcohol of a particular length, and likewise mixtures of (meth)acrylic esters with alcohols of different lengths.

Suitable C1-4 alkyl (meth)acrylates include, for example, methyl (meth)acrylate, ethyl (meth)acrylate, *n*-propyl (meth)acrylate), *iso*-propyl (meth)acrylate, *n*-butyl (meth)acrylate, *iso*-butyl (meth)acrylate and tert-butyl (meth)acrylate. Particularly preferred C₁₋₄ alkyl (meth)acrylates are methyl (meth)acrylate and *n*-butyl (meth)acrylate; methyl methacrylate and *n*-butyl methacrylate are especially preferred.

The C1-3 alkyl (meth)acrylates for use in accordance with the invention are esters of (meth)acrylic acid and straight chain or branched alcohols having 1 to 3 carbon atoms. The term "C1-3 alkyl (meth)acrylates" encompasses individual (meth)acrylic esters with an alcohol of a particular length, and likewise mixtures of (meth)acrylic esters with alcohols of different lengths.

Suitable C1-3 alkyl (meth)acrylates include, for example, methyl (meth)acrylate, ethyl (meth)acrylate, *n*-propyl (meth)acrylate) and *iso*-propyl (meth)acrylate. Particularly preferred C1-3 alkyl (meth)acrylate is methyl (meth)acrylate.

The C10-30 alkyl (meth)acrylates for use in accordance with the invention are esters of (meth)acrylic acid and straight chain or branched alcohols having 10 to 30 carbon atoms. The term "C10-30 alkyl (meth)acrylates" encompasses individual (meth)acrylic esters with an alcohol of a particular length, and likewise mixtures of (meth)acrylic esters with alcohols of different lengths. Suitable C10-30 alkyl (meth)acrylates include, for example, 2-butyloctyl (meth)acrylate, 2-hexyloctyl (meth)acrylate, decyl (meth)acrylate, 2-butyldecyl (meth)acrylate, 2-hexyldecyl (meth)acrylate, 2-octyldecyl (meth)acrylate, undecyl (meth)acrylate, 5-methylundecyl (meth)acrylate, dodecyl (meth)acrylate, 2-methyldodecyl (meth)acrylate, 2-hexyldodecyl (meth)acrylate, 2-octyldodecyl (meth)acrylate, tridecyl (meth)acrylate, 5-methyltridecyl (meth)acrylate, tetradecyl (meth)acrylate, 2-decyltetradecyl (meth)acrylate, pentadecyl (meth)acrylate, hexadecyl (meth)acrylate, 2-methylhexadecyl (meth)acrylate, 2-dodecylhexadecyl (meth)acrylate, heptadecyl (meth)acrylate, 5-isopropylheptadecyl (meth)acrylate, 4*-tert-*butyloctadecyl (meth)acrylate, 5-ethyloctadecyl (meth)acrylate, 3-isopropyloctadecyl (meth)acrylate, octadecyl (meth)acrylate, 2-decyloctadecyl (meth)acrylate, 2-tetradecyloctadecyl (meth)acrylate, nonadecyl (meth)acrylate, eicosyl (meth)acrylate, cetyleicosyl (meth)acrylate, stearyleicosyl (meth)acrylate, docosyl (meth)acrylate and/or eicosyltetratriacontyl (meth)acrylate. 2-decyl-tetradecyl (meth)acrylate, 2-decyloctadecyl (meth)acrylate, 2-dodecyl-1-hexadecyl (meth)acrylate, 1,2-octyl-1-dodecyl (meth)acrylate, 2-tetradecylocadecyl (meth)acrylate, 1,2-tetradecyl-octadecyl (meth)acrylate and 2-hexadecyl-eicosyl (meth)acrylate.

The C12-15 alkyl (meth)acrylates for use in accordance with the invention are esters of (meth)acrylic acid and alcohols having 10 to 15 carbon atoms. The term "C12-15 alkyl (meth)acrylates" encompasses individual (meth)acrylic esters with an alcohol of a particular length, and likewise mixtures of (meth)acrylic esters with alcohols of different lengths.

Suitable C12-15 alkyl (meth)acrylates include, for example, decyl (meth)acrylate, undecyl (meth)acrylate, 5-methylundecyl (meth)acrylate, dodecyl (meth)acrylate, 2-methyldodecyl (meth)acrylate, tridecyl (meth)acrylate, 5-methyltridecyl (methacrylate, tetradecyl (meth)acrylate and/or pentadecyl (meth)acrylate.

Particularly preferred C12-15 alkyl (meth)acrylates are methacrylic esters of a linear C12-14 alcohol mixture (C12-14 alkyl methacrylate).

The C16-20 alkyl (meth)acrylates for use in accordance with the invention are esters of (meth)acrylic acid and alcohols having 16 to 20 carbon atoms. The term "C16-20 alkyl (meth)acrylates" encompasses individual (meth)acrylic esters with an alcohol of a particular length, and likewise mixtures of (meth)acrylic esters with alcohols of different lengths.

Suitable C16-20 alkyl (meth)acrylates include, for example, 2-hexyldecyl (meth)acrylate, 2-octyldecyl (meth)acrylate, undecyl (meth)acrylate, 5-methylundecyl (meth)acrylate and dodecyl (meth)acrylate.

Particularly preferred C16-20 alkyl (meth)acrylates are methacrylic esters of a linear C16-18 alcohol mixture (C16-18 alkyl methacrylate).

The comonomers for use in accordance with the present invention can be selected from the group consisting of styrene monomers having from 8 to 17 carbon atoms, vinyl esters having from 1 to 11 carbon atoms in the acyl group, vinyl ethers having from 1 to 10 carbon atoms in the alcohol group, (di)alkyl fumarates having from 1 to 10 carbon atoms in the alcohol group, (di)alkyl maleates having from 1 to 10 carbon atoms in the alcohol group, dispersing nitrogen-functionalized monomers, and mixtures of these monomers.

Examples of styrene monomers having from 8 to 17 carbon atoms are styrene, substituted styrenes having an alkyl substituent in the side chain, for example alpha-methylstyrene and alphaethylstyrene, substituted styrenes having an alkyl substituent on the ring, such as vinyltoluene and para-methylstyrene, halogenated styrenes, for example monochlorostyrenes, dichlorostyrenes, tribromostyrenes and tetrabromostyrenes; preferred is styrene.

Examples of vinyl esters having from 1 to 11 carbon atoms in the acyl group include vinyl formiate, vinyl acetate, vinyl propionate, vinyl butyrate. Preferred vinyl esters include from 2 to 9, more preferably from 2 to 5 carbon atoms in the acyl group. The acyl group here may be linear or branched.

Examples of vinyl ethers having from 1 to 10 carbon atoms in the alcohol group include vinyl methyl ether, vinyl ethyl ether, vinyl propyl ether, vinyl butyl ether. Preferred vinyl ethers include from 1 to 8, more preferably from 1 to 4 carbon atoms in the alcohol group. The alcohol group here may be linear or branched.

The notation "(di)ester" means that monoesters, diesters and mixtures of esters, especially of fumaric acid and/or of maleic acid, may be used. The (di)alkyl fumarates having from 1 to 10 carbon atoms in the alcohol group include monomethyl fumarate, dimethyl fumarate, monoethyl fumarate, diethyl fumarate, methyl ethyl fumarate, monobutyl fumarate, dibutyl fumarate, dipentyl fumarate and dihexyl fumarate. Preferred (di)alkyl fumarates comprise from 1 to 8, more preferably from 1 to 4 carbon atoms in the alcohol group. The alcohol group here may be linear or branched. The (di)alkyl maleates having from 1 to 10 carbon atoms in the alcohol group include monomethyl maleate, dimethyl maleate, monoethyl maleate, diethyl maleate, methyl ethyl maleate, monobutyl maleate, dibutyl maleate. Preferred (di)alkyl maleates comprise from 1 to 8, more preferably from 1 to 4 carbon atoms in the alcohol group. The alcohol group here may be linear or branched. Examples of dispersing nitrogen-functionalized monomers are aminoalkyl (meth)acrylates, such as N,N-dimethylaminoethyl (meth)acrylate, N,N-dimethylaminopropyl (meth)acrylate, N,N-diethylaminopentyl (meth)acrylate, N,N-dibutylaminohexadecyl (meth)acrylate; aminoalkyl(meth)acrylamides, such as N,N-dimethylaminopropyl(meth)acrylamide; heterocyclic (meth)acrylates, such as 2-(1-imidazolyl)ethyl (meth)acrylate, 2-(4-morpholinyl)ethyl (meth)acrylate, 1-(2-methacryloyloxyethyl)-2-pyrrolidone, N-methacryloylmorpholine, N-methacryloyl-2-pyrrolidinone, N-(2-methacryloyloxyethyl)-2-pyrrolidinone, N-(3-methacryloyloxypropyl)-2-pyrrolidinone; heterocyclic vinyl compounds, such as 2-vinylpyridine, 4-vinylpyridine, 2-methyl-5-vinylpyridine, 3-ethyl-4-vinylpyridine, 2,3-dimethyl-5-vinylpyridine, vinylpyrimidine, vinylpiperidine, 9-vinylcarbazole, 3-vinylcarbazole, 4-vinylcarbazole, 1-vinylimidazole, 2-methyl-1-vinylimidazole, N-vinylpyrrolidone, N-vinylpyrrolidine, 3-vinylpyrrolidine, N-vinylcaprolactam, N-vinylbutyrolactam, vinyloxolane, vinylfuran, vinyloxazoles and hydrogenated vinyloxazoles.

The N-dispersant monomer may specifically be at least one monomer selected from the group consisting of N-vinyl pyrrolidinone, N,N-dimethylaminoethyl methacrylate, and N,N-dimethylaminopropyl methacrylamide.

A further embodiment of the present invention is directed to a lubricating composition comprising the boronic ester-modified polyalkyl (meth)acrylates **A** as outlined further above, wherein the aminophenylboronic acid ester of general formula (I) is selected from the group consisting of 3-aminophenylboronic acid pinacol ester, 4-aminophenylboronic acid pinacol ester, 3-aminophenylboronic acid 1,2-dihydroxybenzene ester, 4-aminophenylboronic acid 1,2-dihydroxybenzene ester, 3-aminophenylboronic acid 1,2-dihydroxycyclohexyl ester and 4-aminophenylboronic acid 1,2-dihydroxycyclohexyl ester, preferably 3-aminophenylboronic acid pinacol ester and 4-aminophenylboronic acid pinacol ester, more preferably 4-aminophenylboronic acid pinacol ester:

A further embodiment of the present invention is directed to a lubricating oil composition comprising the boronic ester-modified polyalkyl (meth)acrylate copolymers **A** as outlined further above, wherein the maleic acid anhydride is grafted.

A further embodiment of the present invention is directed to a lubricating oil composition comprising grafted boronic ester-modified polyalkyl (meth)acrylate copolymers **A** consisting of a base copolymer **A1** and units **A2** that are grafted thereon, wherein the base copolymer **A1** comprises:
(a1) 15% to 40% by weight of C1-4 alkyl (meth)acrylates, preferably selected from methyl methacrylate and butyl methacrylate, more preferably butyl methacrylate;
(a2) 45% to 80% by weight of C10-30 alkyl (meth)acrylates, preferably a mixture of C12-15 alkyl (meth)acrylates and C16-20 alkyl (meth)acrylates, more preferably a mixture of C12-14 alkyl (meth)acrylates and C16-18 alkyl (meth)acrylates; and
(a3) 0% to 20% by weight of comonomers; and
the grafted units **A2** comprise repeating units prepared from:
   (a4) 1% to 3% by weight of copolymerized or grafted maleic acid anhydride; and
   (a5) 2% to 6% by weight of an aminophenylboronic acid ester of general formula (I) wherein **n, R¹** and **R²** are as defined above.

The content of each component (a1), (a2), (a3), (a4) and (a5) is based on the total composition of the boronic ester-modified polyalkyl (meth)acrylate **A.** In a particular embodiment, the proportions of components (a1), (a2), (a3), (a4) and (a5) add up to 100% by weight.

The copolymers used in the lubricating oil composition according to the present invention are characterized by their ability to form association-related thickeners.

### The diol-functionalized polyalkyl (meth)acrylate copolymer B

The diol functionalized polyalkyl (meth)acrylate copolymer **B** comprises at least one diol selected from C2-30 α,β-di-hydroxyalkyl (meth)acrylate, preferably from C2-10 α,β-dihydroxyalkyl (meth)acrylates, preferably selected from the group consisting of 2,3-dihydroxypropyl methacrylate and 5,6-dihydroxyhexyl methacrylate, preferably 2,3-dihydroxypropyl methacrylate.

According to a first favorite embodiment, the diol functionalized polyalkyl (meth)acrylate copolymer **B** comprises from 90% to 98% molar of C1-30 alkyl (meth)acrylates, and from 2% to 10% molar of a C2-30 α,β-di-hydroxyalkyl (meth)acrylate.

According to a second favorite embodiment, the diol functionalized polyalkyl (meth)acrylate copolymer **B** comprises from 1% to 6% by weight of a diol selected from C2-30 α,β-dihydroxyalkyl (meth)acrylates and from 94 to 99% by weight of C1-30 alkyl (meth)acrylates.

According to a favorite embodiment, the diol selected from C2-30 α,β-dihydroxyalkyl (meth)acrylates and the C1-30 alkyl (meth)acrylates represent from 95 to 99 % by weight of monomers composing copolymer B, preferably from 98% to 100% by weight, even more preferably they represent 100% by weight of the monomers composing copolymer **B.**

Advantageously, the polyalkyl (meth)acrylate copolymer **B** comprises the following monomers:

| | |
|---|---|
| (b1) | 15% to 40% by weight of C1-4 alkyl (meth)acrylates, preferably selected from methyl methacrylate and butyl methacrylate, more preferably butyl methacrylate; |
| (b2) | 45% to 80% by weight of C10-30 alkyl (meth)acrylates, preferably a mixture of C12-15 alkyl (meth)acrylates and C16-20 alkyl (meth)acrylates, more preferably a mixture of C12-14 alkyl (meth)acrylates and C16-18 alkyl (meth)acrylates; |
| (b3) | 0% to 20% by weight of comonomers; and |
| (b4) | 1% to 6% by weight of a diol selected from C2-30 α,β-di-hydroxyalkyl (meth)acrylate, preferably from C2-10 α,β-dihydroxyalkyl (meth)acrylates, preferably selected from the group consisting of 2,3-dihydroxypropyl methacrylate and 5,6-dihydroxyhexyl methacrylate, preferably 2,3-dihydroxypropyl methacrylate. |

The content of each component (b1), (b2), (b3) and (b4) is based on the total composition of the polyalkyl (meth)acrylate copolymer **B.** In a particular embodiment, the proportions of components (b1), (b2), (b3) and (b4) add up to 100% by weight.

The weight-average molecular weight of the diol functionalized polyalkyl (meth)acrylate **copolymer B** used in the present invention is preferably in the range of 50,000 to 400,000 g/mol, more preferably in the range of 150,000 to 250,000 g/mol. The number-average molecular weight of the polyalkyl(meth)acrylate copolymers **B** used in the present invention is preferably in the range of 20,000 to 150,000 g/mol, more preferably in the range of 50,000 to 70,000 g/mol.

Preferably, the diol functionalized polyalkyl(meth)acrylate copolymers **B** used in the present invention have a polydipersity index (PDI) M_{w}/Mₙ in the range of 1 to 10, more preferably in the range of 2 to 6, more preferably in the range of 2 to 3.

M_{w} and Mₙ are determined by size exclusion chromatography (SEC) using commercially available polymethylmethacrylate standards. The determination was done by gel permeation chromatography with THF as eluent.

***The proportions of copolymer A and copolymer B in the compositions comprising them***

The favorite proportions of copolymer **A** and copolymer **B** apply to the lubricant compositions and also to the stock solutions (or concentrated solutions) comprising them.

According to a favorite embodiment, the lubricant composition of the present invention comprises
(A) the boronic ester-modified polyalkyl (meth)acrylate copolymer **A,** and
(B) the diol functionalized polyalkyl (meth)acrylate copolymer **B,** in amounts such that the weight ratio (**A**) :(**B**) is 1 :2 to 2 :1, preferably 1 :1,5 to 1,5 :1, even more preferably 1:1.

According to a favorite embodiment, the component aminophenylboronic acid ester of general formula (I) of the boronic ester-modified polyalkyl (meth)acrylate copolymer **A** and the component C2-30 α,β-di-hydroxyalkyl (meth)acrylate of the diol functionalized polyalkyl (meth)acrylate copolymer **B** are present in a molar ratio of 1 :2 to 2 :1, preferably from 1 :1,5 to 1,5 :1, even more preferably of 1:1.

According to a favorite embodiment, the component aminophenylboronic acid ester of general formula (I) of the boronic ester-modified polyalkyl (meth)acrylate copolymer **A** and the component C2-30 α,β-di-hydroxyalkyl (meth)acrylate of the diol functionalized polyalkyl (meth)acrylate copolymer **B** are present in amounts of 2 mol% to 6 mol% of the respective copolymers. According to a favorite embodiment, the lubricant composition of the present invention comprises a mixture of:
(A) a boronic ester-modified polyalkyl (meth)acrylate copolymer **A,** comprising:

| | |
|---|---|
| (a1) | 15% to 40% by weight of C1-4 alkyl (meth)acrylates, preferably selected from methyl methacrylate and butyl methacrylate, more preferably butyl methacrylate; |
| (a2) | 45% to 80% by weight of C10-30 alkyl (meth)acrylates, preferably a mixture of C12-15 alkyl (meth)acrylates and C16-20 alkyl (meth)acrylates, more preferably a mixture of C12-14 alkyl (meth)acrylates and C16-18 alkyl (meth)acrylates; |
| (a3) | 0% to 20% by weight of comonomers; |
| (a4) | 1% to 3% by weight of maleic acid anhydride; and |
| (a5) | 2% to 6% by weight of an aminophenylboronic acid ester of general formula (I) |

wherein **n** denotes an integer 0 to 12, **R¹** and **R²** are as defined above; and
(B) a polyalkyl (meth)acrylate copolymer **B** comprising the following monomers:

| | |
|---|---|
| (b1) | 15% to 40% by weight of C1-4 alkyl (meth)acrylates, preferably selected from methyl methacrylate and butyl methacrylate, more preferably butyl methacrylate; |
| (b2) | 45% to 80% by weight of C10-30 alkyl (meth)acrylates, preferably a mixture of C12-15 alkyl (meth)acrylates and C16-20 alkyl (meth)acrylates, more preferably a mixture of C12-14 alkyl (meth)acrylates and C16-18 alkyl (meth)acrylates; |
| (b3) | 0% to 20% by weight of comonomers; and |
| (b4) | 1% to 6% by weight of a diol selected from C2-30 α,β-di-hydroxyalkyl (meth)acrylate, preferably from C2-10 α,β-dihydroxyalkyl (meth)acrylates, preferably selected from the group consisting of 2,3-dihydroxypropyl methacrylate and 5,6-dihydroxyhexyl methacrylate, preferably 2,3-dihydroxypropyl methacrylate, |

in amounts such that the weight ratio (**A**) :(**B**) is 1 :2 to 2 :1, preferably 1 :1,5 to 1,5 :1, even more preferably 1:1.

According to a favorite embodiment, the component (a5) aminophenylboronic acid ester of general formula (I) of the boronic ester-modified polyalkyl (meth)acrylate copolymer **A** and the component (b4) C2-30 α,β-di-hydroxyalkyl (meth)acrylate of the diol functionalized polyalkyl (meth)acrylate copolymer **B** are present in a molar ratio (a5) : (b4) of 1 :2 to 2 :1, preferably from 1 :1,5 to 1,5 :1, even more preferably of 1:1.

The content of each component (a1), (a2), (a3), (a4) and (a5) is based on the total composition of the boronic ester-modified polyalkyl (meth)acrylate copolymer **A.** In a particular embodiment, the proportions of components (a1), (a2), (a3), (a4) and (a5) add up to 100% by weight.

The content of each component (b1), (b2), (b3) and (b4) is based on the total composition of the polyalkyl (meth)acrylate copolymer **B.** In a particular embodiment, the proportions of components (b1), (b2), (b3) and (b4) add up to 100% by weight.

Advantageously, in the lubricating composition of the present invention, in the mixture as defined further above, component (a5) of the boronic ester-modified polyalkyl (meth)acrylate copolymer **A** and component (b4) of the polyalkyl (meth)acrylate copolymer **B** are present in amounts of 2 mol% to 6 mol% of the respective copolymers.

Advantageously, in the lubricating composition of the present invention, in the mixture as defined further above, component (a5) of the boronic ester-modified polyalkyl (meth)acrylate copolymer **A** and component (b4) of the polyalkyl (meth)acrylate copolymer **B** are present in molar ratio (a5) : (b4) from 1 :2 to 2 :1, more advantageously from 1 :1,5 to 1,5 :1, even more preferably equal to 1. The mixture comprising the above recited amounts of a boronic ester-modified polyalkyl (meth)acrylate copolymer **A** and a polyalkyl (meth)acrylate copolymer **B** can be used to thicken a lubricating oil composition.

### The base oil

The term "oil" means a fatty substance that is liquid at room temperature (25°C) and atmospheric pressure (760 mmHg i.e. 10⁵ Pa).

The term "base oil" or "lubricant oil" means an oil which attenuates the friction between two moving parts in order to facilitate the functioning of these parts. The lubricant oils may be of natural, mineral or synthetic origin.

The lubricant oils of natural origin may be oils of plant or animal origin, preferably oils of plant origin such as rapeseed oil, sunflower oil, palm oil, coconut kernel oil, etc.

The lubricant oils of mineral origin are of petroleum origin and are extracted from petroleum fractions originating from the atmospheric and vacuum distillation of crude oil. The distillation may be followed by refining operations such as solvent extraction, deasphalting, deparaffinning with solvent, hydrotreatment, hydrocracking, hydroisomerization, hydrofinishing, etc. By way of illustration, mention may be made of paraffinic mineral base oils such as the oil Bright Stock Solvent (BSS), naphthenic mineral base oils, aromatic mineral oils, hydrorefined mineral bases whose viscosity index is about 100, hydrocracked mineral bases whose viscosity index is between 120 and 130, or hydroisomerized mineral bases whose viscosity index is between 140 and 150. The lubricant oils of synthetic origin (or synthetic bases) originate, as their name indicates, from chemical synthesis, such as the addition of a product to itself or polymerization, or the addition of one product to another product such as esterification, alkylation, fluorination, etc., of components originating from petrochemistry, carbon chemistry and mineral chemistry such as: olefins, aromatics, alcohols, acids, halogen-based, phosphorus-based, silicon-based compounds, etc. By way of illustration, mention may be made of:
synthetic oils based on synthetic hydrocarbons such as poly-alpha-olefins (PAO), internal polyolefins (IPO), polybutenes and polyisobutenes (PIB), alkylbenzenes and alkylated polyphenyls;
synthetic oils based on esters such as diacid esters or neopolyol esters;
synthetic oils based on polyglycols, such as monoalkylene glycols, polyalkylene glycols and polyalkylene glycol monoethers;
synthetic oils based on phosphate esters;
synthetic oils based on silicon derivatives such as silicone oils or polysiloxanes.

The base oil may also be defined as specified by the American Petroleum Institute (API) (see April 2008 version of "Appendix E-API Base Oil Interchangeability Guidelines for Passenger Car Motor Oils and Diesel Engine Oils", section 1.3 Sub-heading 1.3. "Base Stock Categories").

The API currently defines five groups of lubricant base stocks (API 1509, Annex E - API Base Oil Interchangeability Guidelines for Passenger Car Motor Oils and Diesel Engine Oils, September 2011). Groups I, II and III are mineral oils which are classified by the amount of saturates and sulphur they contain and by their viscosity indices; Group IV are polyalphaolefins; and Group V are all others, including e.g. ester oils. The table below illustrates these API classifications.

| Group | Saturates* | Sulphur content** | Viscosity Index (VI) *** |
|---|---|---|---|
| I | < 90% | > 0.03% | 80-120 |
| II | at least 90% | not more than 0.03% | 80-120 |
| III | at least 90% | not more than 0.03% | at least 120 |
| IV | All polyalphaolefins (PAOs) | | |
| V | All others not included in Groups I, II, III or IV (e.g. ester oils) | | |

| | | | |
|---|---|---|---|
| * measured according to the standard ASTM D2007 ** measured according to the standards ASTM D2622, ASTM D4294, ASTM D4927 and ASTM D3120 *** measured according to the standard ASTM D2270 | | | |

The kinematic viscosity at 100°C (KV100) of appropriate apolar base oils used to prepare a lubricating composition in accordance with the present invention is preferably in the range of 1,5 mm²/s to 150 mm²/s, more preferably in the range of 1,5 mm²/s to 15 mm²/s, according to ASTM D445.

Further base oils which can be used in accordance with the present invention are Group II-III Fischer-Tropsch derived base oils.

Fischer-Tropsch derived base oils are known in the art. By the term "Fischer-Tropsch derived" is meant that a base oil is, or is derived from, a synthesis product of a Fischer-Tropsch process. A Fischer-Tropsch derived base oil may also be referred to as a GTL (Gas-To-Liquids) base oil. Suitable Fischer-Tropsch derived base oils that may be conveniently used as the base oil in the lubricating composition of the present invention are those as for example disclosed in EP 0 776 959, EP 0 668 342, WO 97/21788, WO 00/15736, WO 00/14188, WO 00/14187, WO 00/14183, WO 00/14179, WO 00/08115, WO 99/41332, EP 1 029 029, WO 01/18156, WO 01/57166 and WO 2013/189951.

Especially for engine oil formulations are used base oils of API Group II to V.

### Method of thickening a lubricating oil composition

A further embodiment of the present invention is directed to a method of thickening a lubricating oil composition, comprising the steps of:
(i) preparing a boronic ester-modified polyalkyl (meth)acrylate copolymer **A;**
(ii) mixing the boronic ester-modified polyalkyl (meth)acrylate copolymer **A** of step (i) with a diol functionalized polyalkyl (meth)acrylate **B** to receive a thermo-associative copolymer mixture; and
(iii) applying the thermo-associative copolymer mixture of step (ii) to a lubricating oil composition.

The favorite embodiments recited for the copolymers **A** and **B** and their proportions apply to the method of thickening a lubricating oil composition.

### Lubricating oil composition

Another embodiment of the present invention is directed to a lubricating oil composition, comprising:
(A) 0.1% to 10% by weight of a boronic ester-modified polyalkyl (meth)acrylate copolymer **A,**
(B) 0.1% to 10% by weight of a diol functionalized polyalkyl (meth)acrylate copolymer **B,**
(C) more than 60% to 99.8 % by weight of a base oil, and
(D) 0% to 15% of one or more further additives.

The favorite embodiments recited above for the copolymers **A** and **B,** their combination and their proportions apply to the lubricating oil composition.

The content of each component (A), (B), (C) and (D) is based on the total composition of the lubricating oil composition. In a particular embodiment, the proportions of components (A), (B), (C) and (D) add up to 100% by weight.

The lubricating oil composition according to the invention may also contain, as component (D), further additives selected from the group consisting of conventional VI improvers, dispersants, defoamers, detergents, antioxidants, pour point depressants, antiwear additives, extreme pressure additives, friction modifiers, anticorrosion additives, dyes and mixtures thereof.

Conventional VI improvers include hydrogenated styrene-diene copolymers (HSDs, US4116 917, US3772196 and US4788316), especially based on butadiene and isoprene, and also olefin copolymers (OCPs, K. Marsden: "Literature Review of OCP Viscosity Modifiers", Lubrication Science 1 (1988), 265), especially of the poly(ethylene-co-propylene) type, which may often also be present in N/O-functional form with dispersing action, or PAMAs, which are usually present in N-functional form with advantageous additive properties (*boosters*) as dispersants, wear protection additives and/or friction modifiers (DE 1 520 696 to Röhm and Haas, WO 2006/007934 to RohMax Additives).

Compilations of VI improvers and pour point improvers for lubricant oils, especially motor oils, are detailed, for example, in T. Mang, W. Dresel (eds.): "Lubricants and Lubrication", Wiley-VCH, Weinheim 2001: R. M. Mortier, S. T. Orszulik (eds.): "Chemistry and Technology of Lubricants", Blackie Academic & Professional, London 1992; or J. Bartz: "Additive für Schmierstoffe", Expert-Verlag, Renningen-Malmsheim 1994.

Appropriate dispersants include poly(isobutylene) derivatives, for example poly(isobutylene)succinimides (PIBSIs), including borated PIBSIs; and ethylene-propylene oligomers having N/O functionalities.

Dispersants (including borated dispersants) are preferably used in an amount of 0 to 5% by weight, based on the total amount of the lubricating oil composition.

Suitable defoamers are silicone oils, fluorosilicone oils, fluoroalkyl ethers, etc..

The defoaming agent is preferably used in an amount of 0.005 to 0.1% by weight, based on the total amount of the lubricating oil composition.

The preferred detergents include metal-containing compounds, for example phenoxides; salicylates; thiophosphonates, especially thiopyrophosphonates, thiophosphonates and phosphonates; sulfonates and carbonates. As metal, these compounds may contain especially calcium, magnesium and barium. These compounds may preferably be used in neutral or overbased form.

Detergents are preferably used in an amount of 0.2 to 1% by weight, based on the total amount of the lubricating oil composition.

The suitable antioxidants include, for example, phenol-based antioxidants and amine-based antioxidants.

Phenol-based antioxidants include, for example, octadecyl-3-(3,5-di-tert-butyl-4-hydroxyphenyl)propionate; 4,4' -methylenebis(2,6-di-tert-butylphenol); 4,4' -bis(2,6-di-t-butylphenol); 4,4' -b is(2-methyl-6-t-butylphenol); 2,2' -methylenebis(4-ethyl-6-t-butylphenol); 2,2' - methylenebis( 4-methyl-6-t-butyl phenol); 4,4' -butyl idenebis(3-methyl-6-t-butylphenol); 4,4'-isopropylidenebis(2,6-di-t-butylphenol); 2,2'-methylenebis(4-methyl-6-nonylphenol); 2,2'-isobutylidenebis(4,6-dimethylphenol); 2,2'-methylenebis(4-methyl-6-cyclohexylphenol); 2,6-di-t-butyl-4-methylphenol; 2,6-di-t-butyl-4-ethyl-phenol; 2,4-dimethyl-6-t-butylphenol; 2,6-di-t-amyl-p-cresol; 2,6-di-t-butyi-4-(N,N'-dimethylaminomethylphenol); 4,4'thiobis(2-methyl-6-t-butylphenol); 4,4'-thiobis(3-methyl-6-t-butylphenol); 2,2'-thiobis(4-methyl-6-t-butylphenol); bis(3-methyl-4-hydroxy-5-t-butylbenzyl) sulfide; bis(3,5-di-t-butyl-4-hydroxybenzyl) sulfide; n-octyl-3-(4-hydroxy-3,5-di-t-butylphenyl)propionate; n-octadecyl-3-(4-hydroxy-3,5-di-t-butylphenyl)propionate; 2,2'-thio[diethyl-bis-3-(3,5-di-t-butyl-4-hydroxyphenyl)propionate], etc. Of those, especially preferred are bis-phenol-based antioxidants and ester group containing phenol-based antioxidants.

The amine-based antioxidants include, for example, monoalkyldiphenylamines such as monooctyldiphenylamine, monononyldiphenylamine, etc.; dialkyldiphenylamines such as 4,4' - dibutyldiphenylamine, 4,4'-dipentyldiphe nylamine, 4,4'- dihexyldiphenylamine, 4,4'-diheptyldiphenylamine, 4,4'-dioctyldiphenylamine, 4,4'-dinonyldiphenylamine, etc.; polyalkyldiphenylamines such as tetrabutyldiphenylamine, tetrahexyldiphenylamine, tetraoctyldiphenylamine, tetranonyldiphenylamine, etc.; naphthylamines, concretely alpha-naphthylamine, phenyl-alpha-naphthylamine and further alkyl-substituted phenyl-alpha-naphthylamines such as butylphenyl-alpha-naphthylamine, pentylphenyl-alpha-naphthylamine, hexylphenyl-alpha-naphthylamine, heptylphenyl-alpha-naphthylamine, octylphenyl-alpha-naphthylamine, nonylphenyl-alpha-naphthylamine, etc. Of those, diphenylamines are preferred to naphthylamines, from the viewpoint of the antioxidation effect thereof.

Suitable antioxidants may further be selected from the group consisting of compounds containing sulfur and phosphorus, for example metal dithiophosphates, for example zinc dithiophosphates (ZnDTPs), "OOS triesters" = reaction products of dithiophosphoric acid with activated double bonds from olefins, cyclopentadiene, norbornadiene, α-pinene, polybutene, acrylic esters, maleic esters (ashless on combustion); organosulfur compounds, for example dialkyl sulfides, diaryl sulfides, polysulfides, modified thiols, thiophene derivatives, xanthates, thioglycols, thioaldehydes, sulfur-containing carboxylic acids; heterocyclic sulfur/nitrogen compounds, especially dialkyldimercaptothiadiazoles, 2-mercaptobenzimidazoles; zinc bis(dialkyldithiocarbamate) and methylene bis(dialkyldithiocarbamate); organophosphorus compounds, for example triaryl and trialkyl phosphites; organocopper compounds and overbased calcium- and magnesium-based phenoxides and salicylates.

Antioxidants are used in an amount of 0 to 15% by weight, preferably 0.1 to 10% by weight, more preferably 0.5 to 5% by weight, based on the total amount of the lubricating oil composition.

The pour-point depressants include ethylene-vinyl acetate copolymers, chlorinated paraffinnaphthalene condensates, chlorinated paraffin-phenol condensates, polymethacrylates, polyalkylstyrenes, etc. Preferred are polymethacrylates having a mass-average molecular weight of from 5.000 to 50.000 g/mol.

The amount of the pour point depressant is preferably from 0.1 to 5% by weight, based on the total amount of the lubricating oil composition.

The preferred antiwear and extreme pressure additives include sulfur-containing compounds such as zinc dithiophosphate, zinc di-C₃₋₁₂-alkyldithiophosphates (ZnDTPs), zinc phosphate, zinc dithiocarbamate, molybdenum dithiocarbamate, molybdenum dithiophosphate, disulfides, sulfurized olefins, sulfurized oils and fats, sulfurized esters, thiocarbonates, thiocarbamates, polysulfides, etc.; phosphorus-containing compounds such as phosphites, phosphates, for example trialkyl phosphates, triaryl phosphates, e.g. tricresyl phosphate, amine-neutralized mono- and dialkyl phosphates, ethoxylated mono- and dialkyl phosphates,phosphonates, phosphines, amine salts or metal salts of those compounds, etc.; sulfur and phosphorus-containing anti-wear agents such as thiophosphites, thiophosphates, thiophosphonates, amine salts or metal salts of those compounds, etc.

The antiwear agent may be present in an amount of 0 to 3% by weight, preferably 0.1 to 1.5% by weight, more preferably 0.5 to 0.9% by weight, based on the total amount of the lubricating oil composition.

Friction modifiers used may include mechanically active compounds, for example molybdenum disulfide, graphite (including fluorinated graphite), poly(trifluoroethylene), polyamide, polyimide; compounds that form adsorption layers, for example long-chain carboxylic acids, fatty acid esters, ethers, alcohols, amines, amides, imides; compounds which form layers through tribochemical reactions, for example saturated fatty acids, phosphoric acid and thiophosphoric esters, xanthogenates, sulfurized fatty acids; compounds that form polymer-like layers, for example ethoxylated dicarboxylic partial esters, dialkyl phthalates, methacrylates, unsaturated fatty acids, sulfurized olefins or organometallic compounds, for example molybdenum compounds (molybdenum dithiophosphates and molybdenum dithiocarbamates MoDTCs) and combinations thereof with ZnDTPs, copper-containing organic compounds.

Friction modifiers may be used in an amount of 0 to 6% by weight, preferably 0.05 to 4% by weight, more preferably 0.1 to 2% by weight, based on the total amount of the lubricating oil composition. Some of the compounds listed above may fulfil multiple functions. ZnDTP, for example, is primarily an antiwear additive and extreme pressure additive, but also has the character of an antioxidant and corrosion inhibitor (here: metal passivator/deactivator).

The above-detailed additives are described in detail, inter alia, in T. Mang, W. Dresel (eds.): "Lubricants and Lubrication", Wiley-VCH, Weinheim 2001; R. M. Mortier, S. T. Orszulik (eds.): "Chemistry and Technology of Lubricants".

Preferably, the total concentration of the one or more additives (D) is 0.05% to 15% by weight, more preferably 3% to 10% by weight, based on the total weight of the lubricating oil composition.

### Additive composition

Another embodiment of the present invention is directed to an additive composition, comprising:
(A) 0.1% to 25% by weight of a boronic ester-modified polyalkyl (meth)acrylate copolymer **A,**
(B) 0.1% to 25% by weight of a diol functionalized polyalkyl (meth)acrylate copolymer **B,**
(C) 40% to 60% by weight of a base oil, and
(D) 0.1% to 30% by weight of at least one additive selected from the group consisting of conventional VI improvers, dispersants, defoamers, detergents, antioxidants, pour point depressants, antiwear additives, extreme pressure additives, friction modifiers, anticorrosion additives, dyes and mixtures thereof.

The additive composition, also known as stock solution, or concentrated solution, or mother solution, is used to prepare a lubricating composition, by dilution with a base oil which can be identical to or different from the base oil of the additive composition.

The favorite embodiments recited above for the copolymers **A** and **B** and their proportions apply to the additive composition.

The content of each component (A), (B), (C) and (D) is based on the total composition of additive. In a particular embodiment, the proportions of components (A), (B), (C) and (D) add up to 100% by weight.

### Process for preparing the lubricant and additive compositions of the invention

The lubricant compositions and the additive compositions of the invention are prepared by means that are well known to those skilled in the art. For example, it notably suffices for a person skilled in the art:
- to take a desired amount of a solution comprising the boronic ester-modified polyalkyl (meth)acrylate copolymer **A** as defined above;
- to take a desired amount of a solution comprising the diol functionalized polyalkyl (meth)acrylate copolymer **B** as defined previously;
- optionally to take a desired amount of a solution comprising additives (D) as defined above;
- to mix, either simultaneously or sequentially, the solutions in a lubricant base oil, to obtain the lubricant composition of the invention.

The order of addition of the compounds has no influence in the implementation of the process for preparing the lubricant composition.

Alternately, the lubricating oil composition can be prepared by dilution of a concentrated solution of additives.

### Process for improving the thickening efficiency of a lubricating oil composition

A further embodiment of the present invention is directed to a process for improving the thickening efficiency of a lubricating oil composition by adding a boronic ester-modified polyalkyl (meth)acrylate copolymer **A** and a diol functionalized polyalkyl (meth)acrylate copolymer **B,** comprising the monomers as outlined further above.

### Properties of the lubricating compositions according to the invention

The lubricant compositions of the invention result from the mixing of associative copolymers which have the property of increasing the viscosity of the lubricant oil via associations. The lubricant compositions according to the invention have the advantage in that these associations or crosslinking are reversible.

The boronic ester functionalized copolymers **A** and the diol functionalized copolymers **B** as defined above have the advantage of being associative and of exchanging chemical bonds, notably in a hydrophobic medium, notably an apolar hydrophobic medium.

Under certain conditions, the boronic ester functionalized copolymers **A** and the diol functionalized copolymers **B** as defined above may be crosslinked.

The boronic ester functionalized copolymers **A** and the diol functionalized copolymers **B** also have the advantage of being exchangeable.

The term "associative" means that covalent chemical bonds of boronic ester type are established between the boronic ester functionalized copolymers **A** and the diol functionalized copolymers **B.** Depending on the functionality of the boronic ester functionalized copolymers **A** and the diol functionalized copolymers **B** and depending on the composition of the mixtures, the formation of covalent bonds between boronic ester functionalized copolymers **A** and the diol functionalized copolymers **B** will optionally be able to lead to the formation of a three-dimensional polymer network.

The term "chemical bond" means a covalent chemical bond of boronic ester type.

The term "exchangeable" means that the compounds are capable of exchanging chemical bonds between themselves by transesterification without the total number or nature of the chemical functions being modified.

The lubricant compositions according to the invention have improved thermal stability, an improved viscosity index, improved stability to oxidation, better cycling performance, and better reproducibility of the performance qualities over time, and also better resistance to mechanical degradation.

A person skilled in the art knows how to adjust the various parameters of the various constituents of the composition to obtain a lubricant composition whose viscosity is suitable for use.

The amount of boronic ester bonds that can be established between the diol functionalized copolymers **B** and the boronic ester functionalized copolymers **A** is adjusted by a person skilled in the art by means of an appropriate selection of the diol functionalized copolymers **B,** of the boronic ester functionalized copolymers **A,** and of their amounts.

### Method for obtaining the copolymers used in the lubricating oil composition

The boronic ester-modified polyalkyl (meth)acrylate copolymers **A** and the diol functionalized polyalkyl (meth)acrylate copolymers **B** as disclosed above can be prepared by free-radical polymerization and by related methods of controlled free-radical polymerization, for example ATRP (= atom transfer radical polymerization) or RAFT (= reversible addition fragmentation chain transfer).

Standard free-radical polymerization is detailed, inter alia, in Ullmann's Encyclopedia of Industrial Chemistry, Sixth Edition. In general, a polymerization initiator and optionally a chain transfer agent are used for this purpose.

The usable initiators include azo initiators widely known in the technical field, such as AIBN and 1,1-azobiscyclohexanecarbonitrile, and also peroxy compounds such as methyl ethyl ketone peroxide, acetylacetone peroxide, dilauryl peroxide, tert-butyl per-2-ethylhexanoate, ketone peroxide, tert-butyl peroctoate, methyl isobutyl ketone peroxide, cyclohexanone peroxide, dibenzoyl peroxide, tert-butyl perbenzoate, 2,2-bis(tert-butylperoxy)butane, tert-butyl peroxyisopropylcarbonate, 2,5-bis(2-ethylhexanoylperoxy)-2,5-dimethylhexane, tert-butyl peroxy-2-ethylhexanoate, tert-butyl peroxy-3,5,5-trimethylhexanoate, dicumyl peroxide, 1,1-bis(tert-butylperoxy)cyclohexane, 1,1-bis(tert-butylperoxy)-3,3,5-trimethylcyclohexane, cumyl hydroperoxide, tert-butyl hydroperoxide, bis(4-tert-butylcyclohexyl) peroxydicarbonate, mixtures of two or more of the aforementioned compounds with one another, and mixtures of the aforementioned compounds with unspecified compounds which can likewise form free radicals. Preferably used in accordance with the present invention are tert-butyl perbenzoate and 2,2-bis(tert-butylperoxy)butane. Suitable chain transfer agents are especially oil-soluble mercaptans, for example n-dodecyl mercaptan or 2-mercaptoethanol, or else chain transfer agents from the class of the terpenes, for example terpinolene.

The ATRP method is known per se. It is assumed that this is a "living" free-radical polymerization, but no restriction is intended by the description of the mechanism. In these processes, a transition metal compound is reacted with a compound having a transferable atom group. This involves transfer of the transferable atom group to the transition metal compound, as a result of which the metal is oxidized. This reaction forms a free radical which adds onto ethylenic groups. However, the transfer of the atom group to the transition metal compound is reversible, and so the atom group is transferred back to the growing polymer chain, which results in formation of a controlled polymerization system. It is accordingly possible to control the formation of the polymer, the molecular weight and the molecular weight distribution.

This reaction regime is described, for example, by J.-S. Wang, et al., J. Am. Chem. Soc, vol. 117, p. 5614-5615 (1995), by Matyjaszewski, Macromolecules, vol. 28, p. 7901-7910 (1995). In addition, patent applications WO 96/30421, WO 97/47661, WO 97/18247, WO 98/40415 and WO 99/10387 disclose variants of the above-elucidated ATRP. In addition, the polymers of the invention can also be obtained via RAFT methods, for example. This method is described in detail, for example, in WO 98/01478 and WO 2004/083169.

The polymerization can be conducted under standard pressure, reduced pressure or elevated pressure. The polymerization temperature is also uncritical. In general, however, it is in the range from -20°C to 200°C, preferably 50°C to 150°C and more preferably 80°C to 130°C.

The polymerization can be conducted with or without solvent. The term "solvent" should be understood here in a broad sense. The solvent is selected according to the polarity of the monomers used, it being possible with preference to use 100N oil, comparatively light gas oil and/or aromatic hydrocarbons, for example toluene or xylene.

As outlined further above, the boronic ester-modified polyalkyl (meth)acrylate copolymers **A** comprise either copolymerized or grafted units of maleic acid anhydride.

In cases where the boronic ester-modified polyalkyl (meth)acrylate copolymers **A** are subsequently grafted with maleic acid anhydride, this is preferably done by a polymer-analogous reaction after the above-described preparation of boronic ester-modified polyalkyl (meth)acrylate copolymers **A.** Accordingly, it is possible with preference first to prepare a polymer by the use of reactive polar unsaturated monomers like maleic acid anhydride. The reactive units are subsequently further reacted with an aminophenylboronic acid ester of general formula (I) as described further above. The reaction of the reactive polar unsaturated monomer present in the polymer, preferably of the maleic acid anhydride, with the mentioned aminophenylboronic acid esters can be effected typically between 40°C and 180°C, preferably between 80°C and 180°C and more preferably between 100°C and 160°C. The aminophenylboronic acid ester can preferably be added in an equimolar amount to the reactive polar groups, preferably to the anhydride. If excessive amounts of aminophenylboronic acid ester are added, it can subsequently be removed from the mixture. In the case of excessively small proportions, reactive groups remain, which can optionally be converted to less reactive groups by addition of small amounts of water.

The aminophenylboronic acid ester can be added in pure form to the reaction mixture or in a suitable solvent. Preference is given to polar solvents, especially esters, e.g. butyl acetate, diisononyl adipate or dioctylsebacate.

According to the nature of the reactive reactant group converted, water may be formed. For example, in the case of use of anhydride groups, water is released, which, in a particular aspect of the present invention, can be removed substantially completely from the reaction mixture, it being possible to drive out water, for example, by means of dry nitrogen. In addition, it is possible to use desiccants. Volatile solvents such as butyl acetate, if used, can be distilled off after the reaction, preferably under reduced pressure.

### Figures

The following figures illustrate the results retrieved for the viscosity indices when using the polymers in the compositions of the present invention:
- Figure 1:: Viscosity indices of polymer mixtures A to N (5% of a 1:1 copolymer mixture in Yubase 4+ as base oil) versus solutions of the single copolymers (5% of each polymer in Yubase 4+ as base oil).

The invention is illustrated by the following non-limiting examples.

### Experimental Part

### Abbreviations

- AMA: alkyl methacrylate
- AMBER: 4-aminophenylboronic acid pinacol ester
- BMA: C₄-alkyl methacrylate = *n*-butyl methacrylate
- Diol 1: 2,3-dihydroxypropyl methacrylate (2,3-DHMA)
- Diol 2: 5,6-dihydroxyhexyl methacrylate (5,6-DHMA)
- GPC: gel permeation chromatography
- KV: kinematic viscosity measured according to ASTM D445
- KV40: kinematic viscosity @40°C, measured according to ASTM D7042
- KV100: kinematic viscosity @100°C, measured according to ASTM D7042
- LMA: lauryl methacrylate, 73% C12, 27% C14, all linear
- MAA: maleic acid anhydride
- MMA: C₁-alkyl methacrylate = methyl methacrylate
- Mₙ: number-average molecular weight
- M_{w}: weight-average molecular weight
- NB3043: Nexbase^{®} 3043, Group III base oil from Neste with a KV100 of 4.3 cSt
- PDI: polydispersity index
- SMA: stearyl methacrylate, 6% C14, 30% C16, 64% C18, all linear
- tBPO: tert-butyl-peroxy-2-ethyl-hexanoate
- VI: viscosity index, measured according to ISO 2909
- Yubase 4+: Group III base oil from SK Lubricants with a KV100 of 4.2 cSt

### Test methods

The boronic ester-modified polyalkyl (meth)acrylate copolymers **A** and the diol functionalized polyalkyl (meth)acrylate copolymers **B** were characterized with respect to their molecular weight and PDI.

The weight-average molecular weights (M_{w}) of the boronic ester-modified polyalkyl (meth)acrylates **A** and the diol functionalized polyalkyl (meth)acrylates **B** were determined by gel permeation chromatography (GPC) using polymethyl methacrylate calibration standards according to DIN 55672-1 using the following measurement conditions:

| | |
|---|---|
| Eluent: | tetrahydrofuran (THF), including 0.02 M 2-diethylamino ethylamine |
| Operation temperature: | 35°C |
| Column: | column set consisting of four columns: SDV 106 Å, SDV 104 Å and SDV 103 Å (PSS Standards Service GmbH, Mainz, Germany), all with the size of 300 x 8 mm and an average particle size of 10 µm |
| Flow rate: | 1 mL/min |
| Injected volume: | 100 µL |
| Instrument: | Agilent 1100 series consisting of an autosampler, pump and column oven |
| Detection device: | A refractive index detector from Agilent 1260 series. |

The additive compositions including the boronic ester-modified polyalkyl (meth)acrylate copolymers **A** and the diol functionalized polyalkyl (meth)acrylate copolymers **B** were characterized with respect to their viscosity index (VI) to ASTM D 2270, kinematic viscosity at 40°C (KV40) and 100°C (KV100) to ASTM D445.

In the experimental, the % are expressed by weight of monomers with regards to the total weight of the copolymers unless expressed otherwise.

### Synthesis of the boronic ester-modified polyalkyl (meth)acrylate copolymers A

### (1) Synthesis of the base polymers either for later grafting with maleic acid anhydride or already copolymerized with maleic acid anhydride

Base polymers without maleic acid anhydride: Examples 1a, 2a and 5a

Base polymers with maleic acid anhydride: Examples 3a, 4a and 6a

A solution of 0.8% of initiator 2,2-bis(tert-butylperoxy)butane in the monomer mixture is prepared at room temperature (compositional details of the monomer mixtures are shown in Tables 1 and 2). An apparatus with 4-neck flask and precision glass saber stirrer was initially charged with 300 g NB3043. After heating to 106°C under nitrogen, 450 g of a monomer-initiator-mixture was added within 2 hours. Then the reaction mixture was cooled down to 95°C and 0.4% (based to the total amount of monomers) of 2,2-bis(tert-butylperoxy)butane was added and the resulting mixture stirred at 95°C overnight. 750 g of a 60% solution of polymer in NB3043 was obtained.

**Table 1: Monomer mixtures used to prepare the base polymers for later grafting with maleic acid anhydride.**

| **Example #** | **Type of polymer** | **BMA [%]** | **LMA [%]** | **SMA [%]** |
|---|---|---|---|---|
| 1a | base polymer | 34.61 | 46.43 | 18.96 |
| 2a | base polymer | 26.85 | 51.94 | 21.21 |
| 5a | base polymer | 26.85 | 51.94 | 21.21 |

**Table 2: Monomer mixtures used to prepare the base polymers with copolymerized maleic anhydride.**

| **Example #** | **Type of polymer** | **BMA [%]** | **LMA [%]** | **SMA [%]** | **MAA [%]** |
|---|---|---|---|---|---|
| 3a | MAA copolymer | 34.19 | 45.86 | 18.73 | 1.22 |
| 4a | MAA copolymer | 26.20 | 50.69 | 20.71 | 2.40 |
| 6a | MAA copolymer | 34.19 | 45.86 | 18.73 | 1.22 |

The conversion of the used monomers was around 100%; i.e. the net compositions of the resulting polymers correspond to the mixtures used in the copolymerizations.

### (2) Grafting step before post-polymerization functionalization

### Example 1b (base polymer was Example 1a)

Maleic acid anhydride was heated up at 90°C. An apparatus with a 4-neck flask and precision glass saber stirrer was charged with 400 g of the base polymer mixture as prepared under (1) and heated up to 110°C under nitrogen. Subsequently, 3 g of molten maleic anhydride was added followed by an addition of 1.2 g of tert-butyl perbenzoate. Subsequently, the reaction temperature was increased to 130°C. After 1 hour and 2 hours, another 0.6 g of tert-butyl perbenzoate was each added to the reaction mixture. The mixture was then cooled down to 120°C to add after 3 hours 1 g of 2,2-bis(tert-butylperoxy)butane and after 4 hours 2 g of 2,2-bis(tert-butylperoxy)butane and the mixture is stirred overnight. 408 g of a 60% solution of polymer in NB3043 was obtained.

### Example 2b (base polymer was Example 2a)

Maleic acid anhydride was heated up at 90°C. An apparatus with a 4-neck flask and precision glass saber stirrer was charged with 400 g of the base polymer mixture as prepared under (1) and heated up to 110°C under nitrogen. Then 5.9 g of molten maleic anhydride was added followed by an addition of 1.2 g of tert-butyl perbenzoate. Subsequently, the reaction temperature was increased to 130°C. After 1 hour and 2 hours, another 0.6 g of tert-butyl perbenzoate was each added to the reaction mixture. The mixture was then cooled down to 120°C to add after 3 hours 1 g of 2,2-bis(tert-butylperoxy)butane and after 4 hours 2 g of 2,2-bis(tert-butylperoxy)butane and the mixture is stirred overnight. 411 g of a 60% solution of polymer in NB3043 was obtained.

### Example 5b (base polymer was Example 5a)

Maleic anhydride was heated up at 90°C. An apparatus with a 4-neck flask and precision glass saber stirrer was charged with 500 g of the base polymer mixture as prepared under (1) and heated up to 110°C under nitrogen. Then 7.4 g of molten maleic anhydride was added followed by an addition of 1.5 g of tert-butyl perbenzoate. Subsequently, the reaction temperature was increased to 130°C. After 1 hour and 2 hours, another 0.75 g of tert-butyl perbenzoate was each added to the reaction mixture. The mixture was then cooled down to 120°C to add after 3 hours 1.2 g of 2,2-bis(tert-butylperoxy)butane and after 4 hours 2.4 g of 2,2-bis(tert-butylperoxy)butane and the mixture is stirred overnight. 541 g of a 60% solution of polymer in NB3043 was obtained.

The net compositions of the grafted polymers are shown in the following Table 3.

**Table 3: Net compositions of the grafted polymers.**

| **Example #** | **Type of polymer** | **Base polymer** | **BMA [%]** | **LMA [%]** | **SMA [%]** | **MAA [%]** |
|---|---|---|---|---|---|---|
| 1b | MAA graft polymer | 1a | 34.19 | 45.86 | 18.73 | 1.22 |
| 2b | MAA graft polymer | 2a | 26.20 | 50.69 | 20.71 | 2.40 |
| 5b | MAA graft polymer | 5a | 26.20 | 50.69 | 20.71 | 2.40 |

### (3) Post-polymerization modification

### Example 1c (base polymer was Example 1b)

A solution of 4 wt.% of 4-aminophenylboronic acid pinacol ester in dioctylsebacate was prepared. Then an apparatus with a 4-neck flask, precision glass saber stirrer and condenser was charged with 120 g of the polymer mixture prepared as described under steps (1) or (2). After heating to 130°C under nitrogen, 49.8 g of the 4-aminophenylboronic acid pinacol ester solution was added within 1 hour. The post-grafting reaction was finished 2 hours after the addition of the 4-aminophenylboronic acid pinacol ester and the mixture was diluted to a solids content of 25% with NB3043.

### Example 2c (base polymer was Example 2b)

A solution of 4 wt.% of 4-aminophenylboronic acid pinacol ester in dioctylsebacate was prepared. Then an apparatus with a 4-neck flask, precision glass saber stirrer and condenser was charged with 120 g of the polymer mixture prepared as described under steps (1) or (2). After heating to 130°C under nitrogen, 98.5 g of the 4-aminophenylboronic acid pinacol ester solution was added within 1 hour. The post-grafting reaction was finished 2 hours after the addition of the 4-aminophenylboronic acid pinacol ester and the mixture was diluted to a solids content of 25% with NB3043.

### Example 3b (base polymer was Example 3a)

A solution of 4 wt.% of 4-aminophenylboronic acid pinacol ester in dioctylsebacate was prepared. Then an apparatus with a 4-neck flask, precision glass saber stirrer and condenser was charged with 120 g of the polymer mixture prepared as described under step (1) or (2). After heating to 130°C under nitrogen, 50.2 g of the 4-aminophenylboronic acid pinacol ester solution was added within 1 hour. The post-grafting reaction was finished 2 hours after the addition of the 4-aminophenylboronic acid pinacol ester and the mixture was diluted to a solids content of 25% with NB3043.

### Examples 4b (base polymer was Example 4a)

A solution of 4 wt.% of 4-aminophenylboronic acid pinacol ester in dioctylsebacate was prepared. Then an apparatus with a 4-neck flask, precision glass saber stirrer and condenser was charged with 120 g of the polymer mixture prepared as described under step (1) or (2). After heating to 130°C under nitrogen, 99.5 g of the 4-aminophenylboronic acid pinacol ester solution was added within 1 hour. The post-grafting reaction was finished 2 hours after the addition of the 4-aminophenylboronic acid pinacol ester and the mixture was diluted to a solids content of 25% with NB3043.

### Example 5c (base polymer was Example 5b)

A solution of 4 wt.% of 4-aminophenylboronic acid pinacol ester in dioctylsebacate was prepared. Then an apparatus with a 4-neck flask, precision glass saber stirrer and condenser was charged with 120 g of the polymer mixture prepared as described under step (1) or (2). After heating to 130°C under nitrogen, 98.4 g of the 4-aminophenylboronic acid pinacol ester solution was added within 1 hour. The post-grafting reaction was finished 2 hours after the addition of the 4-aminophenylboronic acid pinacol ester and the mixture was diluted to a solids content of 25% with NB3043.

### Example 6b (base polymer was Example 6a)

A solution of 4 wt.% of 4-aminophenylboronic acid pinacol ester in dioctylsebacate was prepared. Then an apparatus with a 4-neck flask, precision glass saber stirrer and condenser was charged with 120 g of the polymer mixture prepared as described under steps (1) or (2). After heating to 130°C under nitrogen, 49.8 g of the 4-aminophenylboronic acid pinacol ester solution was added within 1 hour. The post-grafting reaction was finished 2 hours after the addition of the 4-aminophenylboronic acid pinacol ester and the mixture was diluted to a solids content of 25% with NB3043.

The net compositions of the resulting boronic ester-modified polyalkyl (meth)acrylates **A** are shown in the following Table 4.

**Table 4: Net compositions of the boronic ester-modified polyalkyl (meth)acrylates A.**

| **Example #** | **Type of polymer** | **Base polymer** | **BMA [%]** | **LMA [%]** | **SMA [%]** | **MAA [%]** | **AMBER [%]** |
|---|---|---|---|---|---|---|---|
| 1c | AMBER graft polymer | 1b | 33.28 | 44.64 | 18.24 | 1.19 | 2.65 |
| 2c | AMBER graft polymer | 2b | 24.87 | 48.11 | 19.65 | 2.28 | 5.09 |
| 3b | AMBER Copolymer | 3a | 33.28 | 44.64 | 18.24 | 1.19 | 2.65 |
| 4b | AMBER Copolymer | 4a | 24.87 | 48.11 | 19.65 | 2.28 | 5.09 |
| 5c | AMBER graft polymer | 5b | 24.87 | 48.11 | 19.65 | 2.28 | 5.09 |
| 6b | AMBER Copolymer | 6a | 33.28 | 44.64 | 18.24 | 1.19 | 2.65 |

### (4) Synthesis of the diol-functionalized base copolymers B

### Examples 7 and 9 (comprising 5,6-DHMA)

### Examples 8 and 10 (comprising 2,3-DHMA)

A solution of a monomer mixture (compositional details of the examples of the used monomer mixtures are given in Table 5) and 0.285% (based to the total amount of monomers) of initiator 2,2-bis(tert-butylperoxy)butane was prepared at room temperature. An apparatus with 4-neck flask and precision glass saber stirrer was initially charged with 60 g butyl acetate. After heating to 106°C under nitrogen, 90 g of the monomer-initiator-mixture was added within 2 hours. Then the reaction mixture was cooled down to 95°C and 0.2% (based to the total amount of monomers) of 2,2-bis(tert-butylperoxy)butane was added and the mixture was stirred at 95°C overnight. 150 g of a 60% solution of polymer in butyl acetate was obtained. The solvent was then exchanged by adding NB3043 to the solution of polymer in butyl acetate. Subsequently, the butyl acetate was removed by vacuum distillation resulting in a 25% solution of polymer in NB3043.

**Table 5: Monomer mixtures used to prepare the diol-functionalized base copolymers B.**

| **Example #** | **BMA [%]** | **LMA [%]** | **SMA [%]** | **DIOL 1 [%]** | **DIOL 2 [%]** |
|---|---|---|---|---|---|
| 7 | 39.00 | 41.54 | 16.96 | | 2.5 |
| 8 | 39.92 | 41.23 | 16.84 | 2.01 | |
| 9 | 34.49 | 43.03 | 17.58 | | 4.9 |
| 10 | 36.30 | 42.42 | 17.32 | 3.96 | |

| | | | | | |
|---|---|---|---|---|---|
| Diol 1 = 2,3-dihydroxypropyl methacrylate Diol 2 = 5,6-dihydroxyhexyl methacrylate | | | | | |

Table 6 shows the net compositions of the working examples and comparative examples. The monomer components will add up to 100%. As the residual monomer content in the retrieved polymers is significantly below 1%, the net compositions of the polymers correspond to the used monomer compositions.

**Table 6: Net compositions of the boronic ester-modified polyalkyl (meth)acrylate copolymers A and the diol functionalized polyalkyl (meth)acrylate copolymers B.**

| **Example #** | **BMA [%]** | **LMA [%]** | **SMA [%]** | **MAA [%]** |
|---|---|---|---|---|
| 1a | 34.61 | 46.43 | 18.96 | |
| 2a | 26.85 | 51.94 | 21.21 | |
| 5a | 26.85 | 51.94 | 21.21 | |
| 3a | 34.19 | 45.86 | 18.73 | 1.22 |
| 4a | 26.20 | 50.69 | 20.71 | 2.40 |
| 6a | 34.19 | 45.86 | 18.73 | 1.22 |
| 1b | 34.19 | 45.86 | 18.73 | 1.22 |
| 2b | 26.20 | 50.69 | 20.71 | 2.40 |
| 5b | 26.20 | 50.69 | 20.71 | 2.40 |

The properties of the boronic ester-modified polyalkyl (meth)acrylates **A** and the polyalkyl (meth)acrylate **B** are presented in the following Table 7.

**Table 7: Properties of the boronic ester-modified polyalkyl (meth)acrylates A and the polyalkyl (meth)acrylate B.**

| **Example #** | **Type of polymer** | **Amount of AMBER [mol%]** | **Amount of diol [mol%]** |
|---|---|---|---|
| 1c | AMBER graft | 2.5 | -- |
| 2c | AMBER graft | 5 | -- |
| 3b | AMBER copolymer | 2.5 | -- |
| 4b | AMBER copolymer | 5 | -- |
| 5c | AMBER graft | 5 | -- |
| 6c | AMBER graft | 2.5 | -- |
| 7 | Diol 2 | -- | 2.5 |
| 8 | Diol 1 | -- | 2.5 |
| 9 | Diol 2 | -- | 5 |
| 10 | Diol 1 | -- | 5 |

The resulting polymers were characterized by their molecular weight and PDI. The results are shown in the following Table 8.

**Table 8: Results of polymer characterization.**

| **Example #** | **Type of polymer** | **M_{w} [g/mol]** | **Mₙ [g/mol]** | **PDI** |
|---|---|---|---|---|
| 1c | AMBER graft | 234,000 | 68,600 | 3.5 |
| 2c | AMBER graft | 486,000 | 63,400 | 5.6 |
| 3b | AMBER copolymer | 111,000 | 55,200 | 2.0 |
| 4b | AMBER copolymer | 110,000 | 53,500 | 2.1 |
| 5c | AMBER graft | 268,000 | 51,200 | 5.2 |
| 6c | AMBER graft | 234,000 | 68,600 | 3.5 |
| 7 | Diol 2 | 165,000 | 54,100 | 3.1 |
| 8 | Diol 1 | 192,000 | 61,000 | 3.2 |
| 9 | Diol 2 | 187,000 | 55,100 | 3.4 |
| 10 | Diol 1 | 191,000 | 63,400 | 3.0 |

The weight-average molecular weights are in the range of 110,000 g/mol (Example 4b) and 486,000 g/mol (Example 2c). The number-average molecular weights are in the range of 51,200 g/mol (Example 5c) and 68,600 g/mol (Examples 1c and 6c).

The thickening efficiency of a VI improver is specified by its KV100 (kinematic viscosity at 100°C) at a given treat rate.

The single polymers were dissolved in a base oil and the retrieved solutions were characterized by their KV40, KV100 and VI. The results are shown in the following Table 9.

**Table 9: Evaluation of compositions comprising 5% polymer in Yubase 4+ as base oil.**

| **Example #** | **Functional group** | **KV40 [mm²/s]** | **KV100 [mm²/s]** | **VI** |
|---|---|---|---|---|
| 1c | AMBER | 8.56 | 34.25 | 244 |
| 2c | AMBER | 10.92 | 43.31 | 256 |
| 3b | AMBER | 7.17 | 29.17 | 225 |
| 4b | AMBER | 6.98 | 28.51 | 222 |
| 5c | AMBER | 8.07 | 33.39 | 229 |
| 6c | AMBER | 8.59 | 34.31 | 244 |
| 7 | Diol 2 | 7.47 | 29.57 | 237 |
| 8 | Diol 1 | 7.83 | 30.74 | 243 |
| 9 | Diol 2 | 7.32 | 29.30 | 232 |
| 10 | Diol 1 | 7.33 | 29.88 | 226 |

It can be seen that the KV40-values are between 6 and 11 mm²/s, the KV100-values are between 28 and 35 mm²/s and the viscosity indices are in the range of 222 (Example 4) and 256 (Example 2).

To show the associative effect of the polymers, mixtures comprising equal parts of an AMBER polymer and a diol-polymer, compositions comprising 5% of a 1:1 polymer mixture in a base oil were prepared and, subsequently, KV40, KV100 and viscosity indices were measured.

The corresponding values are outlined in the following Table 10.

**Table 10: Evaluation of compositions comprising 5% of a 1:1 polymer mixture in Yubase 4+ as base oil.**

| **Mixture #** | **Polymer A** | **Polymer B** | **KV40 [mm²/s]** | **KV100 [mm²/s]** | **VI** |
|---|---|---|---|---|---|
| **A** | **Example 4b** | **Example 9** | **7.31** | **28.92** | **235** |
| | Example 4b | | 6.98 | 28.51 | 222 |
| | | Example 9 | 7.32 | 29.30 | 232 |
| **B** | **Example 4b** | **Example 10** | **7.26** | **28.77** | **234** |
| | Example 4b | | 6.98 | 28.51 | 222 |
| | | Example 10 | 7.33 | 29.88 | 226 |
| **C** | **Example 2c** | **Example 9** | **8.86** | **33.06** | **267** |
| | Example 2c | | 10.92 | 43.31 | 256 |
| | | Example 9 | 7.32 | 29.30 | 232 |
| **D** | **Example 2c** | **Example 10** | **8.56** | **32.35** | **261** |
| | Example 2c | | 10.92 | 43.31 | 256 |
| | | Example 10 | 7.33 | 29.88 | 226 |
| **E** | **Example 3b** | **Example 7** | **7.37** | **29.39** | **233** |
| | Example 3b | | 7.17 | 29.17 | 225 |
| | | Example 7 | 7.47 | 29.57 | 237 |
| **F** | **Example 3b** | **Example 8** | **7.54** | **29.76** | **239** |
| | Example 3b | | 7.17 | 29.17 | 225 |
| | | Example 8 | 7.83 | 30.74 | 243 |
| **G** | **Example 1c** | **Example 7** | **8.31** | **32.17** | **252** |
| | Example 1c | | 8.56 | 34.25 | 244 |
| | | Example 7 | 7.47 | 29.57 | 237 |
| **H** | **Example 1c** | **Example 8** | **8.48** | **32.56** | **255** |
| | Example 1c | | 8.56 | 34.25 | 244 |
| | | Example 8 | 7.83 | 30.74 | 243 |
| **I** | **Example 2c** | **Example 9** | **11.40** | **38.69** | **304** |
| | Example 2c | | 10.92 | 43.31 | 256 |
| | | Example 9 | 7.32 | 29.30 | 232 |
| **J** | **Example 2c** | **Example 10** | **10.81** | **37.94** | **292** |
| | Example 2c | | 10.92 | 43.31 | 256 |
| | | Example 10 | 7.33 | 29.88 | 226 |
| **K** | **Example 6c** | **Example 7** | **8.31** | **32.17** | **252** |
| | Example 6c | | 8.59 | 34.31 | 244 |
| | | Example 7 | 7.47 | 29.57 | 237 |
| **L** | **Example 6c** | **Example 8** | **8.48** | **32.56** | **255** |
| | Example 6c | | 8.59 | 34.31 | 244 |
| | | Example 8 | 7.83 | 30.74 | 243 |
| **M** | **Example 5c** | **Example 9** | **8.86** | **33.06** | **267** |
| | Example 5c | | 8.07 | 33.39 | 229 |
| | | Example 9 | 7.32 | 29.30 | 232 |
| **N** | **Example 5c** | **Example 10** | **8.56** | **32.35** | **261** |
| | Example 5c | | 8.07 | 33.39 | 229 |
| | | Example 10 | 7.33 | 29.88 | 226 |

Table 10 shows that synergistic effects were found for increasing the VI of polymer solutions. The VI of the 1:1 mixture of the polymers was increased versus the VI of the single polymer solutions (see Figure 1). The overall polymer concentration was the same in all solutions.

## Claims

1. Lubricating oil composition, comprising at least:
- more than 60% by weight, based on the total weight of the lubricating composition, of a base oil,
- a boronic ester-modified polyalkyl (meth)acrylate copolymer **A,** comprising 2 mol% to 6 mol% of maleic acid anhydride, and 2 mol% to 6 mol% of an aminophenylboronic acid ester of general formula (I)
wherein n denotes an integer from 0 to 12,
**R¹** and **R²** are independently selected from the group consisting of hydrogen and C1-12 alkyl, or
**R¹** together with **R²** form a ring of general formula (IIa)
wherein **R³, R⁴, R⁵** and **R⁶** are independently selected from the group consisting of H and C1-12 alkyl and the stars "*" represent the bonds to the oxygen atoms, or
**R¹** together with **R²** form a ring of general formula (IIb)
wherein **R³** and **R⁶** are independently selected from the group consisting of H and C1-12 alkyl and the stars "*" represent the bonds to the oxygen atoms, or
**R¹** together with **R²** form a ring of general formula (IIc)
wherein **R⁷** denotes a hydrogen atom or C1-4 alkyl and the stars "*" represent the bonds to the oxygen atoms,
and
- a diol functionalized polyalkyl (meth)acrylate copolymer **B** comprising from 90% to 98% molar of C1-30 alkyl (meth)acrylates, and from 2% to 10% molar of a C2-30 α,β-di-hydroxyalkyl (meth)acrylate.

2. Lubricating oil composition, comprising at least:
- more than 60% by weight, based on the total weight of the lubricating composition, of a base oil,
- a boronic ester-modified polyalkyl (meth)acrylate copolymer **A** comprising from 1% to 3% by weight of copolymerized or grafted maleic acid anhydride; and from 2% to 6% by weight of an aminophenylboronic acid ester of general formula (I)
wherein **n** denotes an integer from 0 to 12,
**R¹** and **R**² are independently selected from the group consisting of hydrogen and C1-12 alkyl, or
**R¹** together with **R²** form a ring of general formula (IIa)
wherein **R³, R⁴, R⁵** and **R⁶** are independently selected from the group consisting of H and C1-12 alkyl and the stars "*" represent the bonds to the oxygen atoms, or
**R¹** together with **R²** form a ring of general formula (IIb)
wherein **R³** and **R⁶** are independently selected from the group consisting of H and C1-12 alkyl and the stars "*" represent the bonds to the oxygen atoms, or
**R¹** together with **R²** form a ring of general formula (IIc)
wherein **R⁷** denotes a hydrogen atom or C1-4 alkyl and the stars "*" represent the bonds to the oxygen atoms,
and
- a diol functionalized polyalkyl (meth)acrylate copolymer **B** comprising from 1% to 6% by weight of a diol selected from C2-30 α,β-dihydroxyalkyl (meth)acrylates.

3. The lubricating oil composition as claimed in claim 1 or in claim 2, wherein it comprises at least:
- from more than 60% to 99.8 % by weight of a base oil;
- from 0.1% to 10% by weight of the boronic ester-modified polyalkyl (meth)acrylate copolymer **A,** and
- from 0.1% to 10% by weight of the diol functionalized polyalkyl (meth)acrylate copolymer **B**

4. The lubricating oil composition as claimed in any one of the preceding claims, wherein the boronic ester-modified polyalkyl (meth)acrylate copolymer **A** comprises:
| | |
|---|---|
| (a1) | 15% to 40% by weight of C1-4 alkyl (meth)acrylates, preferably selected from methyl methacrylate and butyl methacrylate, more preferably butyl methacrylate; |
| (a2) | 45% to 80% by weight of C10-30 alkyl (meth)acrylates, preferably a mixture of C12-15 alkyl (meth)acrylates and C16-20 alkyl (meth)acrylates, more preferably a mixture of C12-14 alkyl (meth)acrylates and C16-18 alkyl (meth)acrylates; |
| (a3) | 0% to 20% by weight of comonomers; |
| (a4) | 1% to 3% by weight of copolymerized or grafted maleic acid anhydride; and |
| (a5) | 2% to 6% by weight of an aminophenylboronic acid ester of general formula (I) |

5. The lubricating oil composition as claimed in any one of claims 1 to 4, wherein in the boronic ester-modified polyalkyl (meth)acrylate copolymer **A,** the aminophenylboronic acid ester of general formula (I) is selected from the group consisting of 3-aminophenylboronic acid pinacol ester, 4-aminophenylboronic acid pinacol ester, 3-aminophenylboronic acid 1,2-dihydroxybenzene ester, 4-aminophenylboronic acid 1,2-dihydroxybenzene ester, 3-aminophenylboronic acid 1,2-dihydroxycyclohexyl ester and 4-aminophenylboronic acid 1,2-dihydroxycyclohexyl ester, preferably 3-aminophenylboronic acid pinacol ester and 4-aminophenylboronic acid pinacol ester, more preferably 4-aminophenylboronic acid pinacol ester.

6. The lubricating oil composition as claimed in any one of claims 1 to 5, wherein the boronic ester-modified polyalkyl (meth)acrylate copolymer **A** has a weight-average molecular weight in the range of 50,000 to 800,000 g/mol, preferably in the range of 100,000 to 600,000 g/mol, determined by gel permeation chromatography (GPC) using polymethyl methacrylate calibration standards according to DIN 55672-1.

7. The lubricating oil composition as claimed in any one of claims 1 to 6, wherein in the boronic ester-modified polyalkyl (meth)acrylate copolymer **A** the maleic acid anhydride is grafted.

8. The lubricating oil composition as claimed in claim 7, wherein the boronic ester-modified polyalkyl (meth)acrylate copolymer **A** consists of a base polymer **A1** and units **A2** that are grafted thereon, wherein the base copolymer **A1** comprises:
(a1) 15% to 40% by weight of C1-4 alkyl (meth)acrylates, preferably selected from methyl methacrylate and butyl methacrylate, more preferably butyl methacrylate;
(a2) 45% to 80% by weight of C10-30 alkyl (meth)acrylates, preferably a mixture of C12-15 alkyl (meth)acrylates and C16-20 alkyl (meth)acrylates, more preferably a mixture of C12-14 alkyl (meth)acrylates and C16-18 alkyl (meth)acrylates; and
(a3) 0% to 20% by weight of co-monomers;
the amount of each component (a1) to (a3) being based on the total composition of the boronic ester-modified polyalkyl (meth)acrylate copolymer **A;** and
the grafted units **A2** comprise repeating units prepared from:
(a4) 1% to 3% by weight of copolymerized or grafted maleic acid anhydride; and
(a5) 2% to 6% by weight of an aminophenylboronic acid ester of general formula (I)
the amount of each component (a4) and (a5) being based on the total composition of the boronic ester-modified polyalkyl (meth)acrylate copolymer **A.**

9. The lubricating oil composition as claimed in any one of claims 1 to 8, wherein the diol functionalized polyalkyl (meth)acrylate copolymer **B** comprises the following monomers:
| | |
|---|---|
| (b1) | 15% to 40% by weight of C1-4 alkyl (meth)acrylates, preferably selected from methyl methacrylate and butyl methacrylate, more preferably butyl methacrylate; |
| (b2) | 45% to 80% by weight of C10-30-alkyl (meth)acrylates, preferably a mixture of C12-15 alkyl (meth)acrylates and C16-20 alkyl (meth)acrylates, more preferably a mixture of C12-14 alkyl (meth)acrylates and C16-18 alkyl (meth)acrylates; |
| (b3) | 0% to 20% by weight of comonomers; and |
| (b4) | 1% to 6% by weight of a diol selected from C2-30 α,β-dihydroxyalkyl (meth)acrylates, preferably C2-10 α,β-dihydroxyalkyl (meth)acrylates, preferably selected from the group consisting of 2,3-dihydroxypropyl methacrylate and 5,6-dihydroxyhexyl methacrylate. |

10. The lubricating oil composition as claimed in any one of claims 1 to 9, wherein the component aminophenylboronic acid ester of general formula (I) of the boronic ester-modified polyalkyl (meth)acrylate copolymer **A** and the component C2-30 α,β-di-hydroxyalkyl (meth)acrylate of the diol functionalized polyalkyl (meth)acrylate copolymer **B** are present in a molar ratio of 1 :2 to 2 :1, preferably from 1 :1,5 to 1,5 :1, even more preferably of 1:1.

11. The lubricating oil composition as claimed in any one of claims 1 to 10, wherein it comprises
(A) the boronic ester-modified polyalkyl (meth)acrylate copolymer **A,** and
(B) the diol functionalized polyalkyl (meth)acrylate copolymer **B,** in amounts such that the weight ratio (**A**) : (**B**) is 1 :2 to 2 :1, preferably 1 :1,5 to 1,5 :1, even more preferably 1:1.

12. An additive composition which can be used for the preparation of a lubricating oil composition according to any one of claims 1 to 11, comprising at least:
(A) 0.1% to 25% by weight of a boronic ester-modified polyalkyl (meth)acrylate copolymer **A,**
(B) 0.1% to 25% by weight of a diol functionalized polyalkyl (meth)acrylate copolymer **B,**
(C) 40% to 60% by weight of a base oil; and
(D) 0.1% to 30% by weight of at least one additive selected from the group consisting of conventional VI improvers, dispersants, defoamers, detergents, antioxidants, pour point depressants, antiwear additives, extreme pressure additives, friction modifiers, anticorrosion additives, dyes and mixtures thereof.

13. Method of thickening a lubricating oil composition, comprising the steps of:
(i) preparing a boronic ester-modified polyalkyl (meth)acrylate copolymer **A;**
(ii) mixing the boronic ester-modified polyalkyl (meth)acrylate copolymer **A** of step (i) with a diol functionalized polyalkyl (meth)acrylate copolymer **B** to form a thermo-associative polymer mixture; and
(iii) introducing the polymer mixture of step (ii) into a lubricating oil composition, Wherein the boronic ester-modified polyalkyl (meth)acrylate copolymer **A,** the diol functionalized polyalkyl (meth)acrylate copolymer **B** and the lubricating oil composition are as defined in any one of claims 1 to 11.

14. A process for reducing the energy losses by mechanical part friction, comprising at least one step of placing a mechanical part in contact with a lubricating oil composition as claimed in any one of claims 1 to 11.

15. A process for reducing the fuel consumption of a vehicle, comprising at least one step of placing a mechanical part of the vehicle engine in contact with a lubricating oil composition as claimed in any one of claims 1 to 11.

## Patentansprüche

1. Schmierölzusammensetzung, die zumindest umfasst:
- zu mehr als 60 Gew.-% ein Basisöl bezogen auf das Gesamtgewicht der Schmierzusammensetzung,
- ein boronestermodifiziertes Polyalkyl(meth)acrylat-Copolymer A, umfassend zu 2 Mol-% bis 6 Mol-% Maleinsäureanhydrid und 2 Mol-% bis 6 Mol-% Aminophenylboronsäureester der allgemeinen Formel (I)
wobei n eine ganze Zahl von 0 bis 12 bezeichnet,
**R¹** und **R²** unabhängig aus der Gruppe ausgewählt sind, die aus Wasserstoff und C1-12-Alkyl besteht, oder
**R¹** zusammen mit **R²** einen Ring der allgemeinen Formel (IIa) bildet
wobei R³, **R⁴, R⁵** und **R⁶** unabhängig aus der Gruppe ausgewählt sind, die aus H und C1-12-Alkyl besteht, und die Sterne "*" die Bindungen an die Sauerstoffatome darstellen, oder
**R¹** zusammen mit **R²** einen Ring der allgemeinen Formel (IIb) bildet wobei **R³** und **R⁶** unabhängig von der Gruppe ausgewählt sind, die aus H und C1-12-Alkyl besteht, und die Sterne "*" die Bindungen an die Sauerstoffatome darstellen, oder
**R¹** zusammen mit **R²** einen Ring der allgemeinen Formel (IIc) bildet
wobei R⁷ ein Wasserstoffatom oder C1-4-Alkyl bezeichnet und die Sterne "*" die Bindungen an die Sauerstoffatome darstellen,
und
- ein diolfunktionalisiertes Polyalkyl(meth)acrylat-Copolymer **B,** umfassend zu 90 Mol-% bis 98 Mol-% C1-30-Alkyl(meth)acrylate und zu 2 Mol-% bis 10 Mol-% ein C2-30-α,β-Di-hydroxyalkyl(meth)acrylat.

2. Schmierölzusammensetzung, die zumindest umfasst:
- zu mehr als 60 Gew.-% ein Basisöl bezogen auf das Gesamtgewicht der Schmierzusammensetzung,
- ein boronestermodifiziertes Polyalkyl(meth)acrylat-Copolymer A, umfassend zu 1 Gew.-% bis 3 Gew.-% copolymerisiertes oder gepfropftes Maleinsäureanhydrid; und zu 2 Gew.-% bis 6 Gew.-% einen Aminophenylboronsäureesters der allgemeinen Formel (I)
wobei n eine ganze Zahl von 0 bis 12 bezeichnet,
**R¹** und **R²** unabhängig aus der Gruppe ausgewählt sind, die aus Wasserstoff und C1-C12-Alkyl besteht, oder
**R¹** zusammen mit **R²** einen Ring der allgemeinen Formel (IIa) bildet
wobei R³, **R⁴, R⁵** und **R⁶** unabhängig von der Gruppe ausgewählt sind, die aus H und C1-12-Alkyl besteht, und die Sterne "*" die Bindungen an die Sauerstoffatome darstellen, oder
**R¹** zusammen mit **R²** einen Ring der allgemeinen Formel (IIb) bildet
wobei R³ und **R⁶** unabhängig von der Gruppe ausgewählt sind, die aus H und C1-12-Alkyl besteht, und die Sterne "*" die Bindungen an die Sauerstoffatome darstellen, oder
**R¹** zusammen mit **R²** einen Ring der allgemeinen Formel (IIc) bildet
wobei R⁷ ein Wasserstoffatom oder C1-4-Alkyl bezeichnet und die Sterne "*" die Bindungen an die Sauerstoffatome darstellen,
und
- ein diolfunktionalisiertes Polyalkyl(meth)acrylat-Copolymer **B,** umfassend zu 1 Gew.-% bis 6 Gew.-% ein Diol, ausgewählt aus C2-30-α,β-Dihydroxyalkyl(meth)acrylaten.

3. Schmierölzusammensetzung nach Anspruch 1 oder Anspruch 2, wobei sie zumindest umfasst:
- zu mehr als 60 Gew.-% bis 99,8 Gew.-% ein Basisöl;
- zu 0,1 Gew.-% bis 10 Gew.-% das boronestermodifizierte Polyalkyl(meth)acrylat-Copolymer A, und
- zu 0,1 Gew.-% bis 10 Gew.-% das diolfunktionalisierte Polyalkyl(meth)acrylat-Copolymer B.

4. Schmierölzusammensetzung nach einem der vorhergehenden Ansprüche, wobei das boronestermodifizierte Polyalkyl(meth)acrylat-Copolymer A umfasst:
a1) zu 15 Gew.-% bis 40 Gew.-% C1-4-Alkyl(meth)acrylate, vorzugsweise ausgewählt aus Methylmethacrylat und Butylmethacrylat, mehr bevorzugt Butylmethacrylat;
(a2) zu 45 Gew.-% bis 80 Gew.-% C10-30-Alkyl(meth)acrylate, vorzugsweise ein Gemisch von C12-15-Alkyl(meth)acrylaten und C16-20-Alkyl(meth)acrylaten, mehr bevorzugt ein Gemisch von C12-14-Alkyl(meth)acrylaten und C16-18-Alkyl(meth)acrylaten;
(a3) zu 0 Gew.-% bis 20 Gew.-% Comonomere;
(a4) zu 1 Gew.-% bis 3 Gew.-% copolymerisiertes oder gepfropftes Maleinsäureanhydrid; und
(a5) zu 2 Gew.-% bis 6 Gew.-% einen Aminophenylboronsäureester der allgemeinen Formel (I)

5. Schmierölzusammensetzung nach einem der Ansprüche 1 bis 4, wobei in dem noronestermodifizierten Polyalkyl(meth)acrylat-Copolymer A der Aminophenylboronsäureester der allgemeinen Formel (I) aus der Gruppe ausgewählt ist, die aus 3-Aminophenylboronsäurepinacolester, 4-Am inophenylboronsäurepinacolester, 3-Aminophenylboronsäure-1,2-dihydroxybenzolester, 4-Aminophenylboronsäure-1,2-dihydroxybenzolester, 3-Aminophenylboronsäure-1,2-dihydroxycyclohexylester und 4-Aminophenylboronsäure-1,2-dihydroxycyclohexylester besteht, vorzugsweise 3-Aminophenylboronsäurepinacolester und 4-Aminophenylboronsäurepinacolester, mehr bevorzugt 4-Aminophenylboronsäurepinacolester.

6. Schmierölzusammensetzung nach einem der Ansprüche 1 bis 5, wobei das boronestermodifizierte Polyalkyl(meth)acrylat-Copolymer A ein gewichtsmittleres Molekulargewicht im Bereich von 50.000 bis 800.000 g/mol aufweist, vorzugsweise im Bereich von 100.000 bis 600.000 g/mol, bestimmt mittels Gelpermeationschromatographie (GPC) unter Verwendung von Polymethylmethacrylat-Kalibrierstandards nach **DIN** 55672-1.

7. Schmierölzusammensetzung nach einem der Ansprüche 1 bis 6, wobei in dem boronestermodifizierten Polyalkyl(meth)acrylat-Copolymer A das Maleinsäureanhydrid gepfropft ist.

8. Schmierölzusammensetzung nach Anspruch 7, wobei das boronestermodifizierte Polyalkyl(meth)acrylat-Copolymer A aus einem Basispolymer A1 und daran gepfropften Einheiten A2 besteht, wobei das Basispolymer A1 umfasst:
(a1) zu 15 Gew.-% bis 40 Gew.-% C1-4-Alkyl(meth)acrylate, vorzugsweise ausgewählt aus Methylmethacrylat und Butylmethacrylat, mehr bevorzugt Butylmethacrylat;
(a2) zu 45 Gew.-% bis 80 Gew.-% C10-30-Alkyl(meth)acrylate, vorzugsweise ein Gemisch von C12-15-Alkyl(meth)acrylaten und C16-20-Alkyl(meth)acrylaten, mehr bevorzugt ein Gemisch von C12-14-Alkyl(meth)acrylaten und C16-18-Alkyl(meth)acrylaten; und
(a3) zu 0 Gew.-% bis 20 Gew.-% Comonomere;
wobei die Menge jeder Komponente (a1) bis (a3) sich auf die Gesamtzusammensetzung des boronestermodifizierten Polyalkyl(meth)acrylat-Copolymers A bezieht, und
die gepfropften Einheiten A2 Wiederholungseinheiten umfassen, hergestellt aus:
(a4) zu 1 Gew.-% bis 3 Gew.-% copolymerisiertes oder gepfropftes Maleinsäureanhydrid; und
(a5) zu 2 Gew.-% bis 6 Gew.-% einen Aminophenylboronsäureester der allgemeinen Formel (I)
wobei die Menge jeder Komponente (a4) und (a5) sich auf die Gesamtzusammensetzung des boronestermodifizierten Polyalkyl(meth)acrylat-Copolymers A bezieht.

9. Schmierölzusammensetzung nach einem der Ansprüche 1 bis 8, wobei das diolfunktionalisierte Polyalkyl(meth)acrylat-Copolymer B folgende Monomere umfasst:
(b1) zu 15 Gew.-% bis 40 Gew.-% C1-4-Alkyl(meth)acrylate, vorzugsweise ausgewählt aus Methylmethacrylat und Butylmethacrylat, mehr bevorzugt Butylmethacrylat;
(b2) zu 45 Gew.-% bis 80 Gew.-% C10-30-Alkyl(meth)acrylate, vorzugsweise ein Gemisch von C12-15-Alkyl(meth)acrylaten und C16-20-Alkyl(meth)acrylaten, mehr bevorzugt ein Gemisch von C12-14-Alkyl(meth)acrylaten und C16-18-Alkyl(meth)acrylaten;
(b3) zu 0 Gew.-% bis 20 Gew.-% Comonomere; und
(b4) zu 1 Gew.-% bis 6 Gew.-% ein Diol, ausgewählt aus C2-30-α,β-Dihydroxyalkyl(meth)acrylaten, vorzugsweise C2-10-α,β-Dihydroxyalkyl(meth)acrylaten, vorzugsweise aus der Gruppe ausgewählt, die aus 2,3-Dihydroxypropylmethacrylat und 5,6-Dihydroxyhexylmethacrylat besteht.

10. Schmierölzusammensetzung nach einem der Ansprüche 1 bis 9, wobei die Komponente Aminophenylboronsäureester der allgemeinen Formel (I) des boronestermodifizierten Polyalkyl(meth)acrylat-Copolymers A und die Komponente C2-30-α,β-Di-hydroxyalkyl(meth)acrylat des diolfunktionalisierten Polyalkyl(meth)acrylat-Copolymers B in einem Molverhältnis von 1:2 bis 2:1, vorzugsweise 1:1,5 bis 1,5:1, noch mehr bevorzugt 1:1, vorliegen.

11. Schmierölzusammensetzung nach einem der Ansprüche 1 bis 10, die umfasst:
(A) das boronestermodifizierte Polyalkyl(meth)acrylat-Copolymer A, und
(B) das diolfunktionalisierte Polyalkyl(meth)acrylat-Copolymer B in Mengen, so dass das Gewichtsverhältnis (A):(B) 1:2 bis 2:1, vorzugsweise 1:1,5 bis 1,5:1, noch mehr bevorzugt 1:1, beträgt.

12. Additivzusammensetzung, die zur Herstellung einer Schmierölzusammensetzung nach einem der Ansprüche 1 bis 11 verwendet werden kann, die zumindest umfasst:
(A) zu 0,1 Gew.-% 25 Gew.-% ein boronestermodifiziertes Polyalkyl(meth)acrylat-Copolymer A,
(B) zu 0,1 Gew.-% bis 25 Gew.-% ein diolfunktionalisiertes Polyalkyl(meth)acrylat-Copolymer B,
(C) zu 40 Gew.-% bis 60 Gew.-% ein Basisöl; und
(D) zu 0,1 Gew.-% bis 30 Gew.-% mindestens ein Additiv, das aus der Gruppe ausgewählt ist, die aus konventionellen VI-verbessernden Mitteln, Dispergiermitteln, Entschäumern, Detergentien, Antioxidantien, stockpunktsenkenden Mitteln, Verschleißschutzadditiven, Extremdruckadditiven, Reibungsmodifikatoren, Korrosionsschutzadditiven, Farbstoffen und Gemischen davon besteht.

13. Verfahren zum Eindicken einer Schmierölzusammensetzung, das die Schritte umfasst:
(i) Herstellen eines boronestermodifizierten Polyalkyl(meth)acrylat-Copolymers A;
(ii) Mischen des boronestermodifizierten Polyalkyl(meth)acrylat-Copolymers A aus Schritt (i) mit einem diolfunktionalisierten Polyalkyl(meth)acrylat-Copolymer B, um ein thermoassoziatives Polymergemisch zu bilden; und
(iii) Einbringen des Polymergemischs aus Schritt (ii) in eine Schmierölzusammensetzung,
wobei das boronestermodifizierte Polyalkyl(meth)acrylat-Copolymer A, das diolfunktionalisierte Polyalkyl(meth)acrylat-Copolymer B und die Schmierölzusammensetzung nach einem der Ansprüche 1 bis 11 sind.

14. Verfahren zum Verringern der Energieverluste durch mechanische Teilereibung, das zumindest einen Schritt des Inkontaktbringens eines mechanischen Teils mit einer Schmierölzusammensetzung nach einem der Ansprüche 1 bis 11 umfasst.

15. Verfahren zum Verringern des Kraftstoffverbrauchs eines Fahrzeugs, das zumindest einen Schritt des Inkontaktbringens eines mechanischen Teils des Fahrzeugmotors mit einer Schmierölzusammensetzung nach einem der Ansprüche 1 bis 11 umfasst.

## Revendications

1. Composition d'huile lubrifiante, comprenant au moins :
- plus de 60 % en poids, par rapport au poids total de la composition lubrifiante, d'une huile de base,
- un copolymère de poly((méth)acrylate d'alkyle) modifié par un ester boronique A, comprenant 2 % en moles à 6 % en moles d'anhydride d'acide maléique et 2 % en moles à 6 % en moles d'un ester d'acide aminophénylboronique de formule générale (I)
dans laquelle n désigne un entier de 0 à 12,
R¹ et R² sont indépendamment choisis dans le groupe constitué par hydrogène et alkyle en C1-12, ou
R¹ conjointement avec R² forment un cycle de formule générale (Ila)
dans laquelle R³, R⁴, R⁵ et R⁶ sont chacun indépendamment choisis parmi H et alkyle en C1-12 et les astérisques « * » représentent les liaisons aux atomes d'oxygène, ou
R¹ conjointement avec R² forment un cycle de formule générale (IIb)
dans laquelle R³ et R⁶ sont indépendamment choisis dans le groupe constitué par H et alkyle en C1-12 et les astérisques « * » représentent les liaisons aux atomes d'oxygène, ou
R¹ conjointement avec R² forment un cycle de formule générale (IIc)
dans lequel R⁷ désigne un atome d'hydrogène ou alkyle en C1-4 et les astérisques « * » représentent les liaisons aux atomes d'oxygène,
et
- un copolymère de poly((méth)acrylate d'alkyle) fonctionnalisé par un diol B comprenant de 90 % à 98 % en moles de (méth)acrylates d'alkyle en C1-30, et de 2% à 10% en moles d'un (méth)acrylate de α,β-di-hydroxyalkyle en C2-30.

2. Composition d'huile lubrifiante, comprenant au moins :
- plus de 60 % en poids, par rapport au poids total de la composition lubrifiante, d'une huile de base,
- un copolymère de poly((méth)acrylate d'alkyle) modifié par un ester boronique A comprenant de 1 % à 3 % en poids d'anhydride d'acide maléique copolymérisé ou greffé ; et de 2 % à 6 % en poids d'un ester d'acide aminophénylboronique de formule générale (I)
dans laquelle n désigne un entier de 0 à 12,
R¹ et R² sont indépendamment choisis dans le groupe constitué par hydrogène et alkyle en C1-12, ou
R¹ conjointement avec R² forment un cycle de formule générale (Ila)
dans laquelle R³, R⁴, R⁵ et R⁶ sont chacun indépendamment choisis parmi H et alkyle en C1-12 et les astérisques « * » représentent les liaisons aux atomes d'oxygène, ou
R¹ conjointement avec R² forment un cycle de formule générale (IIb)
dans laquelle R³ et R⁶ sont indépendamment choisis dans le groupe constitué par H et alkyle en C1-12 et les astérisques « * » représentent les liaisons aux atomes d'oxygène, ou
R¹ conjointement avec R² forment un cycle de formule générale (IIc)
dans lequel R⁷ désigne un atome d'hydrogène ou alkyle en C1-4 et les astérisques « * » représentent les liaisons aux atomes d'oxygène,
et
- un copolymère de poly((méth)acrylate d'alkyle) fonctionnalisé par un diol B comprenant de 1 % à 6 % en poids d'un diol choisi parmi des (méth)acrylates de α,β-dihydroxyalkyle en C2-30.

3. Composition d'huile lubrifiante selon la revendication 1 ou la revendication 2, celle-ci comprenant au moins :
- de plus de 60 % à 99,8 % en poids d'une huile de base ;
- de 0,1 % à 10 % en poids du copolymère de poly((méth)acrylate d'alkyle) modifié par un ester boronique A, et
- de 0,1 % à 10 % en poids du copolymère de poly((méth)acrylate d'alkyle) fonctionnalisé par un diol B.

4. Composition d'huile lubrifiante selon l'une quelconque des revendications précédentes, dans laquelle le copolymère de poly((méth)acrylate d'alkyle) modifié par un ester boronique A comprend :
(a1) 15 % à 40 % en poids de (méth)acrylates d'alkyle en C1-4, de préférence choisis parmi le méthacrylate de méthyle et le méthacrylate de butyle, plus préférablement le méthacrylate de butyle ;
(a2) 45 % à 80 % en poids de (méth)acrylates d'alkyle en C10-30, de préférence un mélange de (méth)acrylates d'alkyle en C12-15 et de (méth)acrylates d'alkyle en C16-20, plus préférablement un mélange de (méth)acrylates d'alkyle en C12-14 et de (méth)acrylates d'alkyle en C16-18 ;
(a3) 0 % à 20 % en poids de comonomères ;
(a4) 1 % à 3 % en poids d'anhydride d'acide maléique copolymérisé ou greffé ; et
(a5) 2 % à 6 % en poids d'un ester d'acide aminophénylboronique de formule générale (I)

5. Composition d'huile lubrifiante selon l'une quelconque des revendications 1 à 4, dans laquelle, dans le copolymère de poly((méth)acrylate d'alkyle) modifié par un ester boronique A, l'ester d'acide aminophénylboronique de formule générale (I) est choisi dans le groupe constitué par l'ester de pinacol d'acide 3-aminophénylboronique, l'ester de pinacol d'acide 4-aminophénylboronique, l'ester de 1,2-dihydroxybenzène d'acide 3-aminophénylboronique, l'ester de 1,2-dihydroxybenzène d'acide 4-aminophénylboronique, l'ester de 1,2-dihydroxycyclohexyle d'acide 3-aminophénylboronique et l'ester de 1,2-dihydroxycyclohexyle d'acide 4-aminophénylboronique, de préférence l'ester de pinacol d'acide 3-aminophénylboronique et l'ester de pinacol d'acide 4-aminophénylboronique, plus préférablement l'ester de pinacol d'acide 4-aminophénylboronique.

6. Composition d'huile lubrifiante selon l'une quelconque des revendications 1 à 5, dans laquelle le copolymère de poly((méth)acrylate d'alkyle) modifié par un ester boronique A a un poids moléculaire moyen en poids dans la plage de 50 000 à 800 000 g/mol, de préférence dans la plage de 100 000 à 600 000 g/mol, déterminé par chromatographie par perméation de gel (GPC) en utilisant des standards d'étalonnage de poly(méthacrylate de méthyle) selon DIN 55672-1.

7. Composition d'huile lubrifiante selon l'une quelconque des revendications 1 à 6, dans laquelle, dans le copolymère de poly((méth)acrylate d'alkyle) modifié par un ester boronique A, l'anhydride d'acide maléique est greffé.

8. Composition d'huile lubrifiante selon la revendication 7, dans laquelle le copolymère de poly((méth)acrylate d'alkyle) modifié par un ester boronique A est constitué d'un polymère de base A1 et de motifs A2 greffés sur celui-ci, le copolymère de base A1 comprenant :
(a1) 15 % à 40 % en poids de (méth)acrylates d'alkyle en C1-4, de préférence choisis parmi le méthacrylate de méthyle et le méthacrylate de butyle, plus préférablement le méthacrylate de butyle ;
(a2) 45 % à 80 % en poids de (méth)acrylates d'alkyle en C10-30, de préférence un mélange de (méth)acrylates d'alkyle en C12-15 et de (méth)acrylates d'alkyle en C16-20, plus préférablement un mélange de (méth)acrylates d'alkyle en C12-14 et de (méth)acrylates d'alkyle en C16-18 ; et
(a3) 0 % à 20 % en poids de comonomères ;
la quantité de chaque composant (a1) à (a3) étant basée sur la composition totale du copolymère de poly((méth)acrylate d'alkyle) modifié par un ester boronique A ; et
les motifs greffés A2 comprennent des motifs de répétition préparés à partir de :
(a4) 1 % à 3 % en poids d'anhydride d'acide maléique copolymérisé ou greffé ; et
(a5) 2 % à 6 % en poids d'un ester d'acide aminophénylboronique de formule générale (I) la quantité de chaque composant (a4) et (a5) étant basée sur la composition totale du copolymère de poly((méth)acrylate d'alkyle) modifié par un ester boronique A.

9. Composition d'huile lubrifiante selon l'une quelconque des revendications 1 à 8, dans laquelle le copolymère de poly((méth)acrylate d'alkyle) fonctionnalisé par un diol B comprend les monomères suivants :
(b1) 15 % à 40 % en poids de (méth)acrylates d'alkyle en C1-4, de préférence choisis parmi le méthacrylate de méthyle et le méthacrylate de butyle, plus préférablement le méthacrylate de butyle ;
(b2) 45 % à 80 % en poids de (méth)acrylates d'alkyle en C10-30, de préférence un mélange de (méth)acrylates d'alkyle en C12-15 et de (méth)acrylates d'alkyle en C16-20, plus préférablement un mélange de (méth)acrylates d'alkyle en C12-14 et de (méth)acrylates d'alkyle en C16-18 ;
(b3) 0 % à 20 % en poids de comonomères ; et
(b4) 1 % à 6 % en poids d'un diol choisi parmi des (méth)acrylates de α,β-dihydroxyalkyle en C2-30, de préférence des (méth)acrylates de α,β-dihydroxyalkyle en C2-10, de préférence choisis dans le groupe constitué par le méthacrylate de 2,3-dihydroxypropyle et le méthacrylate de 5,6-dihydroxyhexyle.

10. Composition d'huile lubrifiante selon l'une quelconque des revendications 1 à 9, dans laquelle le composant ester d'acide aminophénylboronique de formule générale (I) du copolymère de poly((méth)acrylate d'alkyle) modifié par un ester boronique A et le composant (méth)acrylate de α,β-dihydroxyalkyle en C2-30 du copolymère de poly((méth)acrylate d'alkyle) fonctionnalisé par un diol B sont présents dans un rapport molaire de 1:2 à 2:1, de préférence de 1:1,5 à 1,5:1, encore plus préférablement de 1:1.

11. Composition d'huile lubrifiante selon l'une quelconque des revendications 1 à 10, celle-ci comprenant
(A) le copolymère de poly((méth)acrylate d'alkyle) modifié par un ester boronique A, et
(B) le copolymère de poly((méth)acrylate d'alkyle) fonctionnalisé par un diol B, dans des quantités telles que le rapport en poids (A):(B) est de 1:2 à 2:1, de préférence de 1:1,5 à 1,5:1, encore plus préférablement de 1:1.

12. Composition d'additif qui peut être utilisée pour la préparation d'une composition d'huile lubrifiante selon l'une quelconque des revendications 1 à 11, comprenant au moins :
(A) 0,1 % à 25 % en poids d'un copolymère de poly((méth)acrylate d'alkyle) modifié par un ester boronique A,
(B) 0,1 % à 25 % en poids d'un copolymère de poly((méth)acrylate d'alkyle) fonctionnalisé par un diol B,
(C) 40 % à 60 % en poids d'une huile de base ; et
(D) 0,1 % à 30 % en poids d'au moins un additif choisi dans le groupe constitué par des améliorants de l'indice de viscosité conventionnels, des dispersants, des antimousses, des détergents, des antioxydants, des abaisseurs du point d'écoulement, des additifs antiusure, des additifs extrême pression, des modificateurs de friction, des additifs anticorrosion, des colorants et des mélanges de ceux-ci.

13. Procédé d'épaississement d'une composition d'huile lubrifiante, comprenant les étapes de :
(i) préparation d'un copolymère de poly((méth)acrylate d'alkyle) modifié par un ester boronique A ;
(ii) mélange du copolymère de poly((méth)acrylate d'alkyle) modifié par un ester boronique A de l'étape (i) avec un copolymère de poly((méth)acrylate d'alkyle) fonctionnalisé par un diol B pour former un mélange de polymères thermo-associatif ; et
(iii) l'introduction du mélange de polymères de l'étape (ii) dans une composition d'huile lubrifiante,
dans laquelle le copolymère de poly((méth)acrylate d'alkyle) modifié par un ester boronique A, le copolymère de poly((méth)acrylate d'alkyle) fonctionnalisé par un diol B et la composition d'huile lubrifiante sont tels que définis dans l'une quelconque des revendications 1 à 11.

14. Procédé de réduction des pertes d'énergie par frottement de pièces mécaniques, comprenant au moins une étape de mise en contact d'une pièce mécanique avec une composition d'huile lubrifiante selon l'une quelconque des revendications 1 à 11.

15. Procédé de réduction de la consommation de carburant d'un véhicule, comprenant au moins une étape de mise en contact d'une pièce mécanique du moteur du véhicule avec une composition d'huile lubrifiante selon l'une quelconque des revendications 1 à 11.
